



US009389522B2

(12) **United States Patent**  
Takahashi et al.

(10) **Patent No.:** US 9,389,522 B2  
(45) **Date of Patent:** Jul. 12, 2016

(54) **ELECTROPHOTOGRAPHIC PHOTOSENSITIVE MEMBER, PROCESS CARTRIDGE, AND ELECTROPHOTOGRAPHIC APPARATUS**

(71) **Applicant:** CANON KABUSHIKI KAISHA, Tokyo (JP)

(72) **Inventors:** Koji Takahashi, Kashiwa (JP); Naoki Ichihashi, Kashiwa (JP); Kan Tanabe, Toride (JP)

(73) **Assignee:** Canon Kabushiki Kaisha, Tokyo (JP)

(\*) **Notice:** Subject to any disclaimer, the term of this patent is extended or adjusted under 35 U.S.C. 154(b) by 0 days.

(21) **Appl. No.:** 14/935,273

(22) **Filed:** Nov. 6, 2015

(65) **Prior Publication Data**

US 2016/0131984 A1 May 12, 2016

(30) **Foreign Application Priority Data**

Nov. 11, 2014 (JP) ..... 2014-229323  
Oct. 20, 2015 (JP) ..... 2015-206608

(51) **Int. Cl.**

G03G 15/00 (2006.01)  
G03G 5/043 (2006.01)  
G03G 5/06 (2006.01)  
G03G 5/05 (2006.01)

(52) **U.S. Cl.**

CPC ..... G03G 5/043 (2013.01); G03G 5/056 (2013.01); G03G 5/0564 (2013.01); G03G 5/0614 (2013.01); G03G 5/0696 (2013.01)

(58) **Field of Classification Search**

CPC ..... G03G 5/43; G03G 5/056; G03G 5/0564; G03G 5/0614; G03G 5/0696

USPC ..... 399/159  
See application file for complete search history.

(56)

**References Cited**

**U.S. PATENT DOCUMENTS**

|                   |        |              |             |
|-------------------|--------|--------------|-------------|
| 5,449,581 A *     | 9/1995 | Matsui ..... | G03G 5/0696 |
|                   |        |              | 430/58.8    |
| 8,507,161 B2 *    | 8/2013 | Wu .....     | G06G 5/051  |
|                   |        |              | 430/58.8    |
| 2009/0232551 A1 * | 9/2009 | Nagao .....  | G03G 5/056  |
|                   |        |              | 399/159     |
| 2010/0068638 A1 * | 3/2010 | Wu .....     | G03G 5/0696 |
|                   |        |              | 430/58.15   |

**FOREIGN PATENT DOCUMENTS**

|                 |        |
|-----------------|--------|
| JP 07005703 A   | 1/1995 |
| JP 2004004159 A | 1/2004 |
| JP 2013142705 A | 7/2013 |
| JP 2014160238 A | 9/2014 |

\* cited by examiner

*Primary Examiner* — Susan Lee

(74) **Attorney, Agent, or Firm:** Canon U.S.A., Inc., IP Division

(57)

**ABSTRACT**

An electrophotographic photosensitive member includes a charge transport layer containing (α) a charge transporting compound, (β) a binding resin in a proportion in the range of 50% by mass to 200% by mass relative to the mass of the charge transporting compound, (γ) a compound being at least one of xylene and toluene with a content in the range of 0.01% by mass to 2.00% by mass relative to the total mass of the charge transport layer, and (δ) a cycloalkanone with a content in the range of 0.01% by mass to 1.20% by mass relative to the total mass of the charge transport layer.

**20 Claims, 1 Drawing Sheet**





## 1

**ELECTROPHOTOGRAPHIC  
PHOTOSENSITIVE MEMBER, PROCESS  
CARTRIDGE, AND  
ELECTROPHOTOGRAPHIC APPARATUS**

**BACKGROUND OF THE INVENTION**

**1. Field of the Invention**

The present disclosure relates to an electrophotographic photosensitive member, a process cartridge, and an electro-photographic apparatus.

**2. Description of the Related Art**

Electrophotographic apparatus users have recently been being diversified. It is desirable that the electrophotographic apparatus can output more high-quality images than ever without varying image quality over the period of use. Accordingly, it is also desirable that the electrophotographic photosensitive member incorporated in such an electrophotographic apparatus respond to these demands.

For forming high-quality images over a long time from the beginning, Japanese Patent Laid-Open No. 2013-142705 discloses an electrophotographic photosensitive member including a photosensitive layer having a surface layer containing 100 ppm by mass to 2500 ppm by mass of an aromatic hydrocarbon.

For suppressing the degradation of sensitivity, Japanese Patent Laid-Open No. 2004-4159 discloses an electrophotographic photosensitive member including a photosensitive layer containing a saturated alicyclic ketone with a content in the range of 3000 ppm to 50000 ppm relative to the solid content.

For suppressing fluctuations in potential, Japanese Patent Laid-Open No. 7-5703 discloses an electrophotographic photosensitive member including a photoconductive layer (photosensitive layer) containing 0.05% by weight to 10.0% by weight of cyclopentanone.

The applications of electrophotographic apparatuses are expanding. Some of the electrophotographic apparatuses come to be used for quick printing without being limited to use in offices. Accordingly, an electrophotographic photosensitive member suitable for high-speed processes is desired.

When the electrophotographic photosensitive member disclosed in Japanese Patent Laid-Open No. 2013-142705 was used in a high-speed process with substantially the same amount of light for image exposure as in a general process, however, the electrophotographic photosensitive member exhibited poor sensitivity, and a desired light portion potential was not obtained.

The electrophotographic photosensitive members disclosed in Japanese Patent Laid-Open Nos. 2004-4159 and 7-5703 also exhibited the same disadvantage in some cases.

**SUMMARY OF THE INVENTION**

The present disclosure provides a more highly sensitive electrophotographic photosensitive member, and a process cartridge and an electrophotographic apparatus that incorporates the more highly sensitive electrophotographic photosensitive member.

According to an aspect of the present disclosure, there is provided an electrophotographic photosensitive member including a support member, and a charge generating layer and a charge transport layer that are disposed over the support member. The charge transport layer contains: (α) a charge transporting compound; (β) a binding resin in a proportion in the range of 50% by mass to 200% by mass relative to the mass of the charge transporting compound; (γ) a compound

## 2

being at least one of xylene and toluene with a content in the range of 0.01% by mass to 2.00% by mass relative to the total mass of the charge transport layer; and (δ) a cycloalkanone with a content in the range of 0.01% by mass to 1.20% by mass relative to the total mass of the charge transport layer.

According to another aspect of the present disclosure, there is provided a process cartridge capable of being removably attached to an electrophotographic apparatus. The process cartridge includes the above-described electrophotographic photosensitive member and at least one device selected from the group consisting of a charging device, a developing device, a transfer device, and a cleaning device. The electrophotographic photosensitive member and the device are held in one body.

Also, an electrophotographic apparatus is provided. The electrophotographic apparatus includes the above-described electrophotographic photosensitive member, a charging device, an exposure device, a developing device, and a transfer device.

Further features of the present invention will become apparent from the following description of exemplary embodiments with reference to the attached drawing.

**BRIEF DESCRIPTION OF THE DRAWING**

FIGURE is a schematic view of the structure of an electrophotographic apparatus provided with a process cartridge including an electrophotographic photosensitive member according to an embodiment of the invention.

**DESCRIPTION OF THE EMBODIMENTS**

As described above, the electrophotographic photosensitive member disclosed herein includes a support member and photosensitive layers including a charge transport layer over the support member, and the charge transport layer contains the above described components (α), (β), (γ) and (δ). In the following description, components (α), (β), (γ) and (δ) may be referred to as compound α, resin β, compound γ, and compound δ, respectively. The electrophotographic photosensitive member may be simply referred to as the photosensitive member.

The present disclosure features a charge transport layer containing at least either xylene or (compound γ) and cycloalkanone (compound δ) each with a specific content, in comparison with Japanese Patent Laid-Open Nos. 2013-142705, 2004-4159 and 7-5703.

The present inventors assume as below the reason why the charge transfer layer containing compounds γ and δ each with a specific content is effective in providing more highly sensitive electrophotographic photosensitive member.

The present inventors believe that the charge transportability (hole transportability) of the charge transport material (for example, a charge transporting compound having a diphenylamine structure) is enhanced by adding specific amounts of compounds γ and δ to the charge transport layer. Consequently, the charge transport material can transport generated holes to the surface of the charge transport layer even if a latent image is formed by exposure at a low luminous energy, and thus the photosensitive member can exhibit a higher sensitivity than the known photosensitive members.

In order to enhance the hole transportability of the charge transport layer, the ratio of the charge transport material to the binding resin may be increased. The range of variable ratio is however limited in view of the degradation in durability of the photosensitive member and the storage stability of the coating liquid for forming the photosensitive member. According to

the approach disclosed herein, the hole transportability of the charge transport material can be enhanced even if the ratio of the charge transport material to the binding resin in the charge transport layer is the same as in the known photosensitive members.

Compound  $\alpha$

Compound  $\alpha$  is at least one of the charge transport materials. Charge transport materials that can be used in an embodiment of the disclosure include triarylamine compounds, hydrazone compounds, styryl compounds, stilbene compounds, and enamine compounds. These compounds are charge transporting compounds having a diphenylamine structure.



(A) 15



(A-1)

(B)



In general formula (A),  $\text{Ph}^1$  and  $\text{Ph}^2$  each represent substituted or unsubstituted phenyl.

Desirably, compound  $\alpha$  is expressed by any one of formulas (A-1) to (A-9) and has a molecular weight of 3000 or less.

More desirably, compound  $\alpha$  is a charge transport material having a partial structure expressed by the following general formula (B), such as compounds (A-1) to (A-3), (A-5) and (A-6). Compounds (A-1) to (A-3) are particularly desirable.

10

(A-2)



(A-3)

(A-4)



(A-5)

(A-6)



-continued

(A-7)



(A-8)



(A-9)



45

Resin  $\beta$ 

Resin  $\beta$  is a binding resin, and examples thereof include polyester resin, acrylic resin, polyvinylcarbazole resin, phenoxy resin, polycarbonate resin, polyvinyl butyral resin, polystyrene resin, polyvinyl acetate resin, polysulfone resin, polyacrylate resin, vinylidene chloride-acrylonitrile copolymer, and poly(vinyl benzal) resin. These binding resins may be used singly, or may be combined to be used as a mixture or a copolymer.

50

55



(C)



(D)

If a polycarbonate resin is used as the binding resin, a polycarbonate resin having a repeating structural unit expressed by the following general formula (C) is advantageous. If a polyester resin is used as the binding resin, a polyester resin having the repeating structural unit expressed by the following general formula (D) is advantageous.

60

65

In general formula (C), R<sup>11</sup> to R<sup>14</sup> each represent hydrogen or methyl. X<sup>1</sup> represents a single bond, cyclohexylidene, or a divalent group expressed by general formula (E) below. In formula (D), R<sup>21</sup> to R<sup>24</sup> each represent hydrogen or methyl. X<sup>2</sup> represents a single bond, cyclohexylidene, or a divalent group expressed by general formula (E) below. Y<sup>1</sup> represents m-phenylene, p-phenylene, or a divalent group formed by binding two p-phenylene groups with an oxygen atom.



10  
(E)  
15

In general formula (E), R<sup>31</sup> and R<sup>32</sup> each represent hydrogen, methyl, or phenyl. Examples of the repeating structural units of the polycarbonate resin expressed by general formula (C) are as follows:



20  
(C-1)  
25  
(C-2)  
30  
(C-3)



30

35

The polycarbonate resin may be a homopolymer of any one of the repeating structural units (C-1) to (C-8), or a copolymer of any two or more of these repeating structural units. Repeating structural units (C-1), (C-2) and (C-4) are more advantageous.

40 Examples of the repeating structural units of the polyester resin expressed by formula (D) are as follows:



-continued



The polyester resin may be a homopolymer of any one of the repeating structural units (D-1) to (D-9), or a copolymer of any two or more of these repeating structural units. Repeating structural units (D-1), (D-2), (D-3), (D-6), (D-7) and (D-8) are more advantageous.

The polycarbonate resin and the polyester resin can be synthesized by, for example, a known phosgene process. The synthesis may be performed by transesterification.

If the polycarbonate or polyester resin is a copolymer, it may be in any form, such as block copolymer, random copolymer, or alternating copolymer.

The polycarbonate or polyester resin may have a weight average molecular weight in the range of 20000 to 300000, such as 50000 to 250000. The weight average molecular weight mentioned herein refers to the polystyrene-equivalent weight average molecular weight measured by the method disclosed in Japanese Patent Laid-Open No. 2007-79555.

The polycarbonate resin or polyester resin as resin  $\beta$  may be a copolymer having a repeating structure including a siloxane structure in addition to the repeating structural unit expressed by formula (C) or (D). For example, such a structural unit may be expressed by the following formula (F-1) or (F-2). Resin  $\beta$  may have the repeating structural unit expressed by formula (F-3).



The binding resin used in the charge transport layer is not limited to polycarbonate resin or polyester resin and may

have the structure expressed by formula (G-1) shown below. Also, the binding resin may contain a resin having a siloxane structure synthesized by the process described below.



### Synthesis of Siloxane Resin

In 10% sodium hydroxide aqueous solution is dissolved 12.0 g of diol expressed by formula (h-1) shown below. Dichloromethane is added to the resulting solution, followed by stirring, and 15 g of phosgene is blown into the solution over 1 hour while the solution is kept at a temperature in the range of 10°C. to 15°C. When about 70% of the phosgene has been blown, 4.2 g of siloxane derivative expressed by formula (h-2) and 4.0 g of diol expressed by formula (h-3) are added to the solution. After the completion of introducing phosgene, the reaction liquid is violently stirred for emulsification, and then, triethylamine is added. The mixture is stirred for 1 hour. Then, the dichloromethane phase is neutralized with phosphoric acid and further rinsed with water until the pH comes to about 7. Subsequently, the resulting liquid phase is dropped into isopropyl alcohol, and the precipitate is collected by filtration and dried to yield a white polymer (resin A3). The resulting resin A3 has a weight average molecular weight of 20,000.



Table 1 shows examples of resin  $\beta$ .

TABLE 1

| Resin $\beta$<br>(Polycarbonate<br>resin A<br>Polyester resin B<br>Other resin C) | Repeating<br>structural<br>unit | Proportion of<br>repeating<br>structural units<br>(in terms of mass) | Weight average<br>molecular<br>weight (Mw) |
|-----------------------------------------------------------------------------------|---------------------------------|----------------------------------------------------------------------|--------------------------------------------|
| Resin A1                                                                          | C-4                             | 55000                                                                |                                            |
| Resin A2                                                                          | C-4/F-1/F-3                     | 6/1.5/2.5                                                            | 60000                                      |
| Resin A3                                                                          | —                               | —                                                                    | 20000                                      |

TABLE 1-continued

| 5<br>Resin $\beta$<br>(Polycarbonate<br>resin A<br>Polyester resin B<br>Other resin C) | 10<br>Repeating<br>structural<br>unit | 15<br>Proportion of<br>repeating<br>structural units<br>(in terms of mass) | 20<br>Weight average<br>molecular<br>weight (Mw) |
|----------------------------------------------------------------------------------------|---------------------------------------|----------------------------------------------------------------------------|--------------------------------------------------|
| Resin B1                                                                               | D-8                                   | 7/3                                                                        | 100000                                           |
| Resin B2                                                                               | D-1/D-6                               |                                                                            | 120000                                           |
| Resin B3                                                                               | D-1                                   |                                                                            | 120000                                           |
| Resin C1                                                                               | G-1                                   |                                                                            | —                                                |

The charge transport layer may further contain an antioxidant, a UV absorber, a plasticizer, silicone oil, or any other additives, if necessary.

Desirably, the proportion of resin  $\beta$  to compound  $\alpha$  in the charge transport layer is in the range of 50% by mass to 200% by mass. When this proportion is less than 50% by mass, the photosensitive member exhibits low durability; and when the proportion is 200% or more, the photosensitive member exhibits low sensitivity. If the charge transport layer is composed of a single layer, the thickness of the charge transport layer is desirably in the range of 6  $\mu$ m to 40  $\mu$ m, such as in the range of 8  $\mu$ m to 35  $\mu$ m. If the charge transport layer has a multilayer structure, the thickness of the charge transport layer closer to the support member is desirably in the range of 6  $\mu$ m to 30  $\mu$ m, and the thickness of the charge transport layer closer to the surface of the photosensitive member is desirably in the range of 6  $\mu$ m to 10  $\mu$ m.

### Compound $\gamma$

Compound  $\gamma$  is at least one of xylene and toluene. Xylene may be o-xylene, m-xylene, p-xylene, or a mixture of these isomers. In the embodiments of the present disclosure, any xylene may be used. o-Xylene is however advantageous.

In order to produce a satisfactory effect, the content of compound  $\gamma$  in the charge transport layer is in the range of 0.01% by mass to 2.00% by mass, desirably in the range of 0.01% by mass to 1.5% by mass, relative to the total mass of the charge transport layer. More desirably, compound  $\gamma$  contains 50% by mass to 100% by mass of xylene.

### Compound $\delta$

In order to produce a satisfactory effect, the content of compound  $\delta$  in the charge transport layer is in the range of 0.01% by mass to 1.20% by mass relative to the total mass of the charge transport layer. Desirably, compound  $\delta$  may contain at least one of cyclopentanone and cyclohexanone. More desirably, compound  $\delta$  contains 50% by mass to 100% by mass of cyclopentanone, and the proportion of compound  $\delta$  in the charge transport layer is in the range of 0.01% by mass to 0.80% by mass relative to the total mass of the charge transfer layer.

### Contents of Compounds $\gamma$ and $\delta$

As described above, compounds  $\gamma$  and  $\delta$  with specific contents in the charge transport layer enable a more highly sensitive electrophotographic photosensitive member to be provided. The photosensitive member may have two or more charge transport layers. In this instance, it is advantageous that at least one of the charge transport layers contains compounds  $\gamma$  and  $\delta$  with the above contents, and the thickness of this charge transport layer account for 60% or more of the total thickness of the charge transport layers. Desirably, the percentage of compound  $\gamma$  to compound  $\delta$  in this charge transport layer ((content of compound  $\gamma$ /content of compound  $\delta$ ) $\times 100$ ) is in the range of 200% by mass to 9000% by mass. In this percentage, the hole transportability of the charge transport material is enhanced, and a satisfactory effect can be produced.

The contents of compounds  $\gamma$  and  $\delta$  in the charge transport layer can be measured by the following method using a quadrupole GC/MS system TRACE ISQ (manufactured by Thermo Fisher Scientific).

An electrophotographic photosensitive member is cut into a 5 mmx40 mm test piece. The test piece is placed in a vial. TurboMatrix HS 40 Headspace Sampler (manufactured by Perkin Elmer) is set to the conditions: 200° C. in Oven, 205° C. in Loop, and 205° C. in Transfer Line. The gas generated from the test piece is measured by gas chromatography, and the amounts of compounds  $\gamma$  and  $\delta$  in the charge transport layer are determined from a calibration curve.

The mass of the charge transfer layer is calculated from the difference in mass between the test piece taken out the vial and the test piece from which the charge transport layer has been removed. The contents of compounds  $\gamma$  and  $\delta$  relative to the total mass of the charge transport layer are calculated from the mass of the charge transport layer and the measured amounts of compounds  $\gamma$  and  $\delta$ .

The test piece from which the charge transport layer has been removed can be prepared by immersing the test piece taken out of the vial in methyl ethyl ketone for 5 minutes to remove the charge transport layer, and then drying the rest of the test piece at 50° C. for 5 minutes.

#### Structure of Electrophotographic Photosensitive Member

The structure of the electrophotographic photosensitive member of the present disclosure will now be described.

The electrophotographic photosensitive member disclosed herein includes a support member, and a charge generating layer and a charge transport layer that are disposed over the support member. In other words, a multilayer (function-separated) photosensitive layer is defined by the charge generating layer and the charge transport layer. The multilayer photosensitive layer is desirably of a forward type including the charge generating layer and the charge transport layer in that order from the direction of the support member. The charge generating layer may have a multilayer structure, and the charge transport layer may have a multilayer structure.

The support member is desirably electrically conductive (electroconductive support member). The material of the support member may be iron, copper, gold, silver, aluminum, or zinc. Alternatively, the support member may be made of an alloy of some metals of titanium, lead, nickel, tin, antimony, indium, chromium and aluminum, or stainless steel (alloy). There may be used a metal or plastic support member coated with a film formed of, for example, aluminum, aluminum alloy or indium oxide-tin oxide alloy by vacuum deposition.

The support member may be a plastic or paper sheet impregnated with electrically conductive particles, such as carbon black, tin oxide particles, titanium oxide particles, or silver particles, or a member made of an electrically conductive binding resin sheet.

The surface of the support member may be cut, roughened or anodized so as to suppress interference fringes caused by scattering of a laser beam.

In order to suppress such interference fringes or to cover flaws in the support member, an electroconductive layer may be formed between the support member and an undercoat layer described later. The electroconductive layer may be formed by applying onto a surface a coating liquid for forming the electroconductive layer prepared by dispersing carbon black, an electrically conductive pigment, a resistance-adjusting pigment and a binding resin in a solvent, and drying the coating film. The coating liquid for the electroconductive layer may contain a compound capable of being cured by, for example, heating or exposure to UV light or radiation

Examples of the binding resin used in the electroconductive layer include acrylic resin, allyl resin, alkyd resin, ethyl cellulose resin, ethylene-acrylic acid copolymer, epoxy resin, casein resin, silicone resin, gelatin resin, phenol resin, butyral resin, polyacrylate resin, polyacetal resin, polyamide-imide resin, polyamide resin, polyallyl ether resin, polyimide resin, polyurethane resin, polyester resin, polycarbonate resin, and polyethylene resin.

Examples of the electrically conductive pigment or the resistance-adjusting pigment include metal (alloy) particles, such as those of aluminum, zinc, copper, chromium, nickel, silver, and stainless steel, and plastic particles coated with any one of these metals. Metal oxide particles may be used, such as those of zinc oxide, titanium oxide, tin oxide, antimony oxide, indium oxide, bismuth oxide, tin-doped indium oxide, or antimony- or tantalum-doped tin oxide.

These pigments may be used singly or in combination. The electrically conductive pigment and the resistance-adjusting pigment may be surface-treated. Exemplary surface treatment agents include a surfactant, a silane coupling agent, and a titanium coupling agent.

In order to reduce light scattering, silicone resin fine particles or acrylic resin fine particles may be added. In addition, the electroconductive layer may further contain other additives, such as a leveling agent, a dispersant, an antioxidant, an ultraviolet absorber, a plasticizer, and a rectifying material.

The thickness of the electroconductive layer may be in the range of 0.2  $\mu\text{m}$  to 40  $\mu\text{m}$ , such as 1  $\mu\text{m}$  to 35  $\mu\text{m}$  or 5  $\mu\text{m}$  to 30  $\mu\text{m}$ .

An undercoat layer (intermediate layer) may be provided between the support member or the electroconductive layer and the photosensitive layer (charge generating layer, charge transport layer) so as to improve the adhesion of the photosensitive layer and improve the injection of charges from the support member. The undercoat layer may be formed by applying an undercoat liquid prepared by mixing a binding resin and a solvent and drying the coating film of the undercoat liquid.

Examples of the binding resin used in the undercoat layer include polyvinyl alcohol, polyethylene oxide, ethyl cellulose, methyl cellulose, casein, polyamide (nylon 6, nylon 66, nylon 610, copolymerized nylon, and N-alkoxymethylated nylon), polyurethane resin, acrylic resin, allyl resin, alkyd resin, phenol resin, and epoxy resin.

The undercoat layer may have a thickness in the range of 0.05  $\mu\text{m}$  to 40  $\mu\text{m}$ . The undercoat layer may further contain metal oxide particles. The metal oxide particles used in the undercoat layer desirably contain particles of at least one metal oxide selected from the group consisting of titanium oxide, zinc oxide, tin oxide, zirconium oxide, and aluminum oxide. Particles containing zinc oxide are advantageous.

The metal oxide particles may be surface-treated with a surface treatment agent, such as a silane coupling agent. The materials can be dispersed using, for example, a homogenizer, an ultrasonic disperser, a ball mill, a sand mill, a roll mill, a vibration mill, an attritor, or a high-speed liquid collision disperser.

The undercoat layer may further contain organic resin particles or a leveling agent so as to, for example, control the surface roughness thereof or reduce cracks therein. The organic resin particles may be hydrophobic organic particles, such as silicone particles, or hydrophilic organic particles, such as cross-linked poly(methacrylate) resin (PMMA) particles.

The undercoat layer may contain other additives, such as a metal, an electrically conductive material, an electron trans-

## 15

porting material, a metal chelate compound, and a silane coupling agent or any other organic compounds.

The charge generating layer may be formed by applying a coating liquid for the charge generating layer prepared by dispersing a charge generation material and a binding resin in a solvent, and drying the coating film of the coating liquid. Alternatively, the charge generating layer may be a deposition film formed by depositing a charge generating material.

Examples of the charge generating material include azo pigments, phthalocyanine pigments, indigo pigments, perylene pigments, polycyclic quinone pigments, squarylium dyes, thiapyrylium salts, triphenylmethane dyes, quinacridone pigments, azulениum salt pigments, cyanine dyes, anthanthrone pigments, pyranthrone pigments, xanthene dyes, quinonimine dyes, and styryl dyes.

These charge generating materials may be used singly or in combination. From the viewpoint of sensitivity, oxytitanium phthalocyanine, chlorogallium phthalocyanine, and hydroxygallium phthalocyanine are advantageous. Crystalline hydroxygallium phthalocyanine whose CuK $\beta$  X-ray diffraction spectrum shows peaks at Bragg angle 20 of  $7.4^\circ \pm 0.3^\circ$  and  $28.2^\circ \pm 0.3^\circ$  is more advantageous.

Examples of the binding resin used in the charge generating layer include polycarbonate resin, polyester resin, butyral resin, polyvinyl acetal resin, acrylic resin, vinyl acetate resin, and urea resin. Among these, butyral resin is advantageous. These binding resins may be used singly, or may be combined to be used as a mixture or a copolymer.

The materials can be dispersed using, for example, a homogenizer, an ultrasonic disperser, a ball mill, a sand mill, a roll mill, or an attritor.

The proportion of the charge generating material in the charge generating layer is desirably in the range of 0.3 parts by mass to 10 parts by mass relative to 1 part by mass of the binding resin. The charge generating layer may further contain a sensitizer, a leveling agent, a dispersant, an antioxidant, a UV absorbent, a plasticizer, and a rectifying material, if necessary. The thickness of the charge generating layer is desirably in the range of 0.01  $\mu\text{m}$  to 5  $\mu\text{m}$ , such as in the range of 0.1  $\mu\text{m}$  to 2  $\mu\text{m}$ .

The charge transport layer is disposed on the charge generating layer. The charge transport layer may be formed by applying a coating liquid for the charge transport layer prepared by dispersing a charge transport material and a binding resin in a solvent, and drying the coating film of the coating liquid.

Examples of the charge transport material include pyrene compounds, N-alkyl carbazole compounds, N,N-dialkylamine compounds, diphenylamine compounds, triphenylamine compounds, triphenylmethane compounds, pyrazoline compounds, and butadiene compounds, in addition to the above-cited compounds, such as triarylamine compounds, hydrazone compounds, and styryl compounds. These charge transport materials may be used singly or in combination. From the viewpoint of preventing cracks in the charge transport layer, compounds having the above-described partial structure expressed by general formula (A) are advantageous. More advantageously, the charge transport material contains any of the compounds expressed by formulas (A-1) to (A-9).

The binding resin used in the charge transport layer, that is, resin  $\beta$ , may be a polycarbonate resin (resin A) having a repeating structural unit expressed by general formula (C) or a polyester resin (resin B) having a repeating structural unit expressed by general formula (D). These binding resins may be used together with acrylic resin, polyvinylcarbazole resin, phenoxy resin, polyvinyl butyral resin, polystyrene resin, polyvinyl acetate resin, polysulfone resin, vinylidene chloride-acrylonitrile copolymer, and poly(vinyl benzal) resin. These binding resins may be used singly, or may be combined to be used as a mixture or a copolymer.

## 16

The solvent used in the coating liquid for the charge transport layer may be an alcohol-based solvent, a sulfoxide-based solvent, a ketone-based solvent, an ether-based solvent, an ester-based solvent, or an aromatic hydrocarbon.

5 The charge transport layer may further contain an antidegradant, a UV absorbent, a plasticizer, a leveling agent, organic fine particles, or inorganic fine particles, if necessary.

Examples of the antidegradant include a hindered phenol-based antioxidant, a hindered amine-based light stabilizer, a 10 sulfur-containing antioxidant, and a phosphorus-containing antioxidant.

The organic fine particles may be fluorine-containing 15 organic resin fine particles, polystyrene fine particles, polyethylene resin particles, or any other polymer resin particles. The inorganic fine particles may be particles of silica or metal oxide such as alumina.

The charge transport layer may be covered with a protective layer so as to increase the abrasion resistance and cleanability of the electrophotographic photosensitive member. The protective layer may be formed by applying a coating liquid for the protective layer prepared by dissolving a binding resin in a solvent, and drying the coating film of the coating liquid.

20 Examples of the binding resin used in the protective layer include polyvinyl butyral resin, polyester resin, polycarbonate resin, polyamide resin, polyimide resin, polyurethane resin, and phenol resin.

Alternatively, the protective layer may be formed by applying a coating solution for the protective layer prepared by dissolving a polymerizable monomer or oligomer in a solvent, and curing the coating film of the coating solution by a 30 crosslinking reaction or a polymerization reaction. The polymerizable monomer or oligomer may be a compound having a chain-polymerizable functional group, such as acryloyloxy or styryl, or a compound having a sequentially polymerizable functional group, such as hydroxy, alkoxy, isocyanate, or epoxy.

35 Examples of the reaction for curing the protective layer include radical polymerization, ionic polymerization, thermal polymerization, photopolymerization, radiation-induced polymerization (electron beam polymerization), plasma CVD, and optical CVD.

The protective layer may further contain electrically conductive particles or charge transport material. The electrically conductive particles may be the same as those used in the electroconductive layer. The charge transport material may be 40 the same as that used in the charge transport layer.

From the viewpoint of abrasion resistance and charge transportability, a charge transport material having a polymerizable functional group is advantageously used. The polymerizable functional group may be acryloyloxy. A charge transport material having two or more polymerizable functional group in the molecule is advantageous.

The surface layer (the charge transport layer or the protective layer) of the electrophotographic photosensitive member may contain organic resin particles or inorganic particles. The 45 organic resin particles may be fluorine-containing organic resin fine particles or acrylic resin particles. The inorganic particles may be those of alumina, silica or titania. Furthermore, the surface layer may contain electrically conductive particles, an antioxidant, a UV absorbent, a plasticizer, a leveling agent, or the like.

50 The thickness of the protective layer may be in the range of 0.1  $\mu\text{m}$  to 30  $\mu\text{m}$ , such as in the range of 1  $\mu\text{m}$  to 10  $\mu\text{m}$ .

The coating liquid for each layer may be applied by dip coating, spray coating, spinner coating, roller coating, Mayer bar coating, blade coating, or any other coating technique.

55 Process Cartridge and Electrophotographic Apparatus FIGURE schematically shows the structure of an electrophotographic apparatus provided with a process cartridge

including an electrophotographic photosensitive member. This electrophotographic photosensitive member **1**, which is cylindrical, is driven for rotation on a shaft **2** in the direction indicated by an arrow at a predetermined peripheral speed (process speed). The surface of the electrophotographic photosensitive member **1** driven for rotation is uniformly charged to a predetermined positive or negative potential with a charging device **3** (primary charging device such as charging roller). Subsequently, an electrostatic latent image corresponding to desired image information is formed on the surface of the charged electrophotographic photosensitive member **1** by irradiation with exposure light (light for exposing images) **4** from an exposure device (image exposing device, not shown). The exposure light **4** has been intensity-modulated according to the time-series electric digital image signals of desired image information output from an image exposure device for, for example, slit exposure or laser beam scanning exposure.

The electrostatic latent image formed on the surface of the electrophotographic photosensitive member **1** is developed (normally developed or reversely developed) into a toner image with a developer (toner) contained in a developing device **5**. The toner image on the surface of the electrophotographic photosensitive member **1** is transferred to a transfer medium **P** by a transfer bias from a transfer device **6**, such as a transfer roller. At this time, the transfer medium **P** is fed to an abutting portion between the electrophotographic photosensitive member **1** and the transfer device **6** from a transfer medium feeder (not shown) in synchronization with the rotation of the electrophotographic photosensitive member **1**. Also, a bias voltage having an opposite polarity to the charge of the toner is applied to the transfer device from a bias source (not shown).

The transfer medium **P** to which the toner image has been transferred is separated from the surface of the electrophotographic photosensitive member **1** and transferred to a fixing device **8** for fixing the toner image, thus being ejected as an image-formed article (printed matter or copy).

The surface of the electrophotographic photosensitive member 1 from which the toner image has been transferred is cleaned with a cleaning device 7 to remove therefrom the developer (toner) or the like remaining after transfer.

Some of the components of the electrophotographic apparatus including the electrophotographic photosensitive member 1, the charging device 3, the developing device 5, and the cleaning device 7 may be integrated in a container as a process cartridge. The process cartridge may be removably mounted to the body of an electrophotographic apparatus. For example, the electrophotographic photosensitive member 1

and at least one selected from among the charging device 3, the developing device 5 and the cleaning device 7 are integrated into a cartridge.

If the electrophotographic apparatus is a copy machine or a printer, the exposure light 4 may be reflected light from or transmitted light through an original image. Alternatively, the exposure may be performed by laser beam scanning according to the signals generated by reading the original image with a sensor, or performed with light emitted by driving an LED array or a liquid crystal shutter array.

## EXAMPLES

The present disclosure will be further described in detail with reference to specific examples. The term "part(s)" used hereinafter refers to "part(s) by mass".

## Preparation of Electrophotographic Photosensitive Member Preparation of Photosensitive Member A-1

An aluminum cylinder of 30 mm in diameter and 357.5 mm in length was used as a support member (cylindrical support member).

Then, in a ball mill were dispersed 60 parts of tin oxide-coated barium sulfate particles (PASTRAN PC1, produced by "Mitsui Mining & Smelting), 15 parts of tin oxide particles (TITANIX JR, produced by Tayca), 43 parts of resol-type phenol resin (PHENOLITE J-325, produced by DIC, solid content: 70% by mass), 0.015 part of silicone oil (SH28PA, produced by Toray Silicone), 3.6 parts of silicone resin particles (TOSPEARL 120, produced by Toray Silicone), 50 parts of 2-methoxy-1-propanol, and 50 parts of methanol for 20 hours to yield a coating liquid for the electroconductive layer. This coating liquid was applied to the surface of the support member by dip coating. The resulting coating film was dried and cured by heating at 140° C. for 1 hour to yield a 15  $\mu\text{m}$  thick electroconductive layer.

Subsequently, 10 parts of copolymerized nylon (Amilan CM8000, produced by Toray) and 30 parts of methoxymethylated 6-nylon resin (Tresin EF-30T, produced by Teikoku Chemical) were dissolved in a mixed solution of 400 parts of methanol and 200 parts of n-butanol to yield a coating liquid for forming an undercoat layer. This coating liquid was applied to the surface of the electroconductive layer by dip coating. The resulting coating film was dried at 100° C. for 30 minutes to yield a 0.45  $\mu\text{m}$  thick undercoat layer.

Subsequently, a sand mill containing glass bead of 1 mm in diameter was charged with 20 parts of a crystalline hydroxygallium phthalocyanine (charge generating material) whose CuK $\beta$  X-ray diffraction spectrum has strong peaks at Bragg angles 20 of  $7.4^\circ \pm 0.2^\circ$  and  $28.2^\circ \pm 0.2^\circ$ , 0.2 part of a calixarene compound expressed by the following formula (1), 10 parts of a polyvinyl butyral (S-LEC BX-1, produced by Sekisui Chemical) and 600 parts of cyclohexanone.



After the materials were dispersed in each other for 4 hours, 700 parts of ethyl acetate was added to the dispersion to yield a coating liquid for forming a charge generating layer. The coating liquid for the charge generating layer was applied to the surface of the undercoat layer by dip coating. The resulting coating film was dried at 80° C. for 15 minutes to yield a 0.17  $\mu\text{m}$  thick charge generating layer.

Subsequently, a coating liquid for a charge transport layer was prepared by mixing:

7.2 parts of the compound expressed by formula (A-1) (charge transporting compound or hole transporting compound);

0.8 part of the compound expressed by formula (A-2) (charge transporting compound or hole transporting compound);

10 parts of resin B1;

16 parts of o-xylene;

28 parts of cyclopentanone; and

36 parts of dimethoxymethane (methylal).

The coating liquid for the charge transport layer was applied to a surface of the charge generating layer by dip coating. The resulting coating film was dried at 120° C. for 60 minutes to yield a 30  $\mu\text{m}$  thick charge transport layer.

Thus, an electrophotographic photosensitive member having a charge transport layer as the surface layer was completed. The resulting electrophotographic photosensitive member was cut into a test piece with the above-mentioned dimensions, and the test piece was subjected to gas chromatography for determination of the contents of o-xylene (compound  $\gamma$ ) and cyclopentanone (compound  $\delta$ ). The o-xylene (compound  $\gamma$ ) content was 1.2% by mass, and the cyclopentanone (compound  $\delta$ ) content was 0.11% by mass. Details of the electrophotographic photosensitive member are shown in Table 2. The resulting electrophotographic photosensitive member was evaluated as Photosensitive member A-1.

Preparation of Photosensitive Members A-2 to A-35

Electrophotographic photosensitive members were prepared in the same process as photosensitive member A-1, except that the contents of resin  $\beta$  and compound  $\gamma$  were varied according to Table 2 and that the drying temperature and drying time were set as shown in Table 3. Details are shown in Tables 2 and 3. The resulting electrophotographic photosensitive members were evaluated as photosensitive members A-2 to A-35, respectively.

Preparation of Photosensitive Members A-101 to A-110

Electrophotographic photosensitive members were prepared in the same process as photosensitive member A-1, except that the contents of resin  $\beta$  and compound  $\gamma$  were varied according to Table 4 and that the drying temperature and drying time were set as shown in Table 5. Details are shown in Tables 4 and 5. The resulting electrophotographic photosensitive members were evaluated as photosensitive members A-101 to A-110, respectively.

Preparation of Photosensitive Members B-1 to B-30

Electrophotographic photosensitive members were prepared in the same process as photosensitive member A-1, except that the contents of compound  $\alpha$ , resin  $\beta$  and compounds  $\gamma$  and  $\delta$  were varied according to Table 6 and that the drying temperature and drying time were set as shown in Table 7. Details are shown in Tables 6 and 7. The resulting electrophotographic photosensitive members were evaluated as Photosensitive members B-1 to B-30, respectively.

Preparation of Photosensitive Members B-101 to B-110

Electrophotographic photosensitive members were prepared in the same process as photosensitive member A-1, except that the contents of compound  $\alpha$ , resin  $\beta$  and compounds  $\gamma$  and  $\delta$  were varied according to Table 8 and that the drying temperature and drying time were set as shown in

Table 9. Details are shown in Tables 8 and 9. The resulting electrophotographic photosensitive members were evaluated as photosensitive members B-101 to B-110, respectively.

Preparation of Photosensitive Members C-1 to C-30

5 Electrophotographic photosensitive members were prepared in the same process as photosensitive member A-1, except that the contents of compound  $\alpha$ , resin  $\beta$  and compounds  $\gamma$  and  $\delta$  were varied according to Table 10 and that the drying temperature and drying time were set as shown in Table 11. Details are shown in Tables 10 and 11. The resulting electrophotographic photosensitive members were evaluated as photosensitive members C-1 to C-30, respectively.

Preparation of Photosensitive Members C-101 to C-110

15 Electrophotographic photosensitive members were prepared in the same process as photosensitive member A-1, except that the contents of compound  $\alpha$ , resin  $\beta$  and compounds  $\gamma$  and  $\delta$  were varied according to Table 12 and that the drying temperature and drying time were set as shown in Table 13. Details are shown in Tables 12 and 13. The resulting electrophotographic photosensitive members were evaluated as photosensitive members C-101 to C-110, respectively.

Preparation of Photosensitive Members D-1 to D-9

20 Electrophotographic photosensitive members were prepared in the same process as photosensitive member A-1, except that the contents of compound  $\alpha$  and the content thereof, resin  $\beta$  and the content thereof, and the contents of compounds  $\gamma$  and  $\delta$  were varied according to Table 14, and that the drying temperature and drying time were set as shown in Table 15. Details are shown in Tables 14 and 15. The resulting electrophotographic photosensitive members were evaluated as photosensitive members D-1 to D-9, respectively.

25 Preparation of Photosensitive Members D-101 to D-109

25 Electrophotographic photosensitive members were prepared in the same process as photosensitive member A-1, except that the charge transport layer was formed to a thickness of 20  $\mu\text{m}$  with the composition in which compound  $\alpha$  and the content thereof, resin  $\beta$  and the content thereof, and the contents of compounds  $\gamma$  and  $\delta$  were varied according to Table 16, and that the drying temperature and drying time were set as shown in Table 17. Details are shown in Tables 16 and 17. The resulting electrophotographic photosensitive members were evaluated as photosensitive members D-101 to D-109, respectively.

30 Preparation of Photosensitive Member D-110

30 The layers up to the charge generating layer were formed in the same manner as in the process of photosensitive member A-1.

35 Then, a coating liquid for a charge transport layer was prepared by mixing the following materials:

10 parts of the compound expressed by the following formula (Z-1) (charge transporting compound or hole transporting compound);  
55 10 parts of resin Al; and  
100 parts of tetrahydrofuran.

40 The coating liquid for the charge transport layer was applied to a surface of the charge generating layer by dip coating. The resulting coating film was dried at 135° C. for 20 minutes to yield a 22  $\mu\text{m}$  thick charge transport layer.

45 Then, a coating liquid for a second charge transport layer was prepared by mixing the following materials:

3 parts of alumina (AA03, produced by Sumitomo Chemical, 60 average primary particle size: 0.3  $\mu\text{m}$ );  
0.06 part of unsaturated carboxylic acid polymer (BYK-P104, produced by BYK);

4 parts of the compound expressed by formula (A-3) (charge transporting compound or hole transporting compound);  
10 parts of resin Al;  
10 parts of o-xylene;  
220 parts of tetrahydrofuran; and  
70 parts of cyclopentanone.

The coating liquid for the charge transport layer was applied to a surface of the charge generating layer by spray coating. The resulting coating film was dried at 135° C. for 20 minutes to yield a 5  $\mu$ m thick second charge transport layer. The resulting electrophotographic photosensitive member was evaluated as photosensitive member D-110.

Part of the second charge transport layer was cut out and placed in a vial. TurboMatrix HS 40 Headspace Sample (manufactured by Perkin Elmer) was set to the conditions: 200° C. in Oven, 205° C. in Loop, and 205° C. in Transfer

10 parts of o-xylene;  
220 parts of tetrahydrofuran; and  
70 parts of cyclopentanone.

5 The coating liquid for the charge transport layer was applied to a surface of the charge generating layer by spray coating. The resulting coating film was dried at 135° C. for 20 minutes to yield a 5  $\mu$ m thick second charge transport layer.

10 The resulting electrophotographic photosensitive member  
10 was evaluated as photosensitive member D-111. The contents  
of compounds  $\gamma$  and  $\delta$  were determined in the same manner as  
those in photosensitive member D-110. The contents of com-  
15 pounds  $\gamma$  and  $\delta$  were 0.006% and 0.004%, respectively. The  
percentage of the compound  $\gamma$  content to the compound  $\delta$   
15 content was 150% by mass.



Line, and the gas generated from the test piece was subjected to gas chromatography. The amounts of compounds  $\gamma$  and  $\delta$  in the charge transport layer were determined from a calibration curve. The mass of the charge transport layer was calculated from the difference between the total mass of the vial after the measurement and the test piece of the charge transport layer and the mass of the vial measured in advance. The contents of compounds  $\gamma$  and  $\delta$  were 0.006% and 0.004%, respectively. The percentage of the compound  $\gamma$  content to the compound  $\delta$  content was 150% by mass.

### Preparation of Photosensitive Member D-111

The layers up to the charge generating layer were formed in the same manner as in the process of photosensitive member A-1.

A coating liquid for a charge transport layer was prepared by mixing the following materials:

10 parts of the compound (Z-1) (charge transfer compound);  
10 parts of resin Al; and  
100 parts of tetrahydrofi-

100 parts of tetrahydrofuran.

The coating liquid for the charge transport layer was applied to a surface of the charge generating layer by dip coating. The resulting coating film was dried at 135° C. for 20 minutes to yield a 22  $\mu\text{m}$  thick charge transport layer.

A coating liquid for a second charge transport layer was prepared by mixing the following materials:

- 3 parts of alumina (AA03, produced by Sumitomo Chemical, average primary particle size: 0.3  $\mu\text{m}$ );
- 0.06 part of unsaturated carboxylic acid polymer (BYK-P104, produced by BYK);
- 4 parts of the compound expressed by formula (Z-2) (charge transporting compound or hole transporting compound);
- 10 parts of resin Al;



## Preparation of Photosensitive Members E-1 to E-9

Electrophotographic photosensitive members were prepared in the same process as photosensitive member A-1, except that the charge transport layer was formed to a thickness of 20  $\mu\text{m}$  with the composition in which compound  $\alpha$  and the content thereof, resin  $\beta$  and the content thereof, and the contents of compounds  $\gamma$  and  $\delta$  were varied according to Table 18, and that the drying temperature and drying time were set as shown in Table 19. Details are shown in Tables 18 and 19. The resulting electrophotographic photosensitive members were evaluated as photosensitive members E-1 to E-9, respectively.

## Preparation of Photosensitive Members E-101 to E-109

Electrophotographic photosensitive members were prepared in the same process as photosensitive member A-1, except that the charge transport layer was formed to a thickness of 20  $\mu\text{m}$  with the composition in which compound  $\alpha$  and the content thereof, resin  $\beta$  and the content thereof, and the contents of compounds  $\gamma$  and  $\delta$  were varied according to Table 20, and that the drying temperature and drying time were set as shown in Table 21. Details are shown in Tables 20 and 21.

The resulting electrophotographic photosensitive members were evaluated as photosensitive members E-101 to E-109, respectively.

Preparation of Photosensitive Members F-1 to F-7

Electrophotographic photosensitive members were prepared in the same process as photosensitive member A-1, except that the charge transport layer was formed to a thickness of 20  $\mu\text{m}$  with the composition in which compound  $\alpha$  and the content thereof, resin  $\beta$  and the content thereof, the content of compounds  $\gamma$ , and compound  $\delta$  and the content thereof were varied according to Table 22, and that the drying temperature and drying time were set as shown in Table 23. Details are shown in Tables 22 and 23. The resulting electrophotographic photosensitive members were evaluated as photosensitive members F-1 to F-7, respectively.

Preparation of Photosensitive Members F-101 to F-109

Electrophotographic photosensitive members were prepared in the same process as photosensitive member A-1, except that the charge transport layer was formed to a thickness of 20  $\mu\text{m}$  with the composition in which compound  $\alpha$  and the content thereof, resin  $\beta$  and the content thereof, the content of compounds  $\gamma$ , and compound  $\delta$  and the content thereof were varied according to Table 24, and that the drying temperature and drying time were set as shown in Table 25. Details are shown in Tables 24 and 25. The resulting electro-

photographic photosensitive members were evaluated as photosensitive members F-101 to F-109, respectively.

Preparation of Photosensitive Member G-1

An electrophotographic photosensitive member was prepared in the same process as photosensitive member A-1, except that the charge transport layer was formed to a thickness of 20  $\mu\text{m}$  with the composition in which compound  $\alpha$  and the content thereof, resin  $\beta$  and the content thereof, compound  $\gamma$  and the content thereof, and compound  $\delta$  and the content thereof were varied according to Table 26, and that the drying temperature and drying time were set as shown in Table 27. Details are shown in Tables 26 and 27. The resulting electrophotographic photosensitive member was evaluated as photosensitive member G-1.

Preparation of Photosensitive Member G-101

An electrophotographic photosensitive member was prepared in the same process as photosensitive member A-1, except that the charge transport layer was formed to a thickness of 20  $\mu\text{m}$  with the composition in which compound  $\alpha$  and the content thereof, resin  $\beta$  and the content thereof, compound  $\gamma$  and the content thereof, and compound  $\delta$  and the content thereof were varied according to Table 28, and that the drying temperature and drying time were set as shown in Table 29. Details are shown in Tables 28 and 29. The resulting electrophotographic photosensitive member was evaluated as photosensitive member G-101. "Xylene" in the following Tables represents "o-xylene".

TABLE 2

|                            | $\alpha$               | $\beta$             | $\gamma$                        | $\delta$          | Another solvent   |                   |    |          |    |
|----------------------------|------------------------|---------------------|---------------------------------|-------------------|-------------------|-------------------|----|----------|----|
|                            | Parts by Compound mass | Parts by Resin mass | content/<br>( $\alpha$ )<br>100 | Parts by Compound | Parts by Compound | Parts by Compound |    |          |    |
| Photosensitive member A-1  | A-1/A-2 7.2/0.8        | Resin 10 B2         | 125                             | Xylene            | 16                | Cyclopentanone    | 28 | Methylal | 36 |
| Photosensitive member A-2  | A-1/A-2 7.2/0.8        | Resin 10 B2         | 125                             | Xylene            | 21                | Cyclopentanone    | 23 | Methylal | 36 |
| Photosensitive member A-3  | A-1/A-2 7.2/0.8        | Resin 10 B2         | 125                             | Xylene            | 16                | Cyclopentanone    | 30 | Methylal | 36 |
| Photosensitive member A-4  | A-1/A-2 7.2/0.8        | Resin 10 B2         | 125                             | Xylene            | 21                | Cyclopentanone    | 25 | Methylal | 36 |
| Photosensitive member A-5  | A-1/A-2 7.2/0.8        | Resin 10 B2         | 125                             | Xylene            | 8                 | Cyclopentanone    | 38 | Methylal | 36 |
| Photosensitive member A-6  | A-1/A-2 7.2/0.8        | Resin 10 B2         | 125                             | Xylene            | 14                | Cyclopentanone    | 38 | Methylal | 36 |
| Photosensitive member A-7  | A-1/A-2 7.2/0.8        | Resin 10 B2         | 125                             | Xylene            | 41                | Cyclopentanone    | 5  | Methylal | 36 |
| Photosensitive member A-8  | A-1/A-2 7.2/0.8        | Resin 10 B2         | 125                             | Xylene            | 41                | Cyclopentanone    | 5  | Methylal | 36 |
| Photosensitive member A-9  | A-1/A-2 7.2/0.8        | Resin 10 B2         | 125                             | Xylene            | 33                | Cyclopentanone    | 13 | Methylal | 36 |
| Photosensitive member A-10 | A-1/A-2 7.2/0.8        | Resin 10 B2         | 125                             | Xylene            | 21                | Cyclopentanone    | 23 | Methylal | 36 |
| Photosensitive member A-11 | A-1/A-2 7.2/0.8        | Resin 10 B2         | 125                             | Xylene            | 16                | Cyclopentanone    | 28 | Methylal | 36 |
| Photosensitive member A-12 | A-1/A-2 7.2/0.8        | Resin 10 B2         | 125                             | Xylene            | 41                | Cyclopentanone    | 20 | Methylal | 36 |
| Photosensitive member A-13 | A-1/A-2 7.2/0.8        | Resin 10 B2         | 125                             | Xylene            | 16                | Cyclopentanone    | 30 | Methylal | 36 |
| Photosensitive member A-14 | A-1/A-2 7.2/0.8        | Resin 10 B2         | 125                             | Xylene            | 2                 | Cyclopentanone    | 40 | Methylal | 36 |
| Photosensitive member A-15 | A-1/A-2 7.2/0.8        | Resin 10 B2         | 125                             | Xylene            | 41                | Cyclopentanone    | 35 | Methylal | 36 |
| Photosensitive member A-16 | A-1/A-2 7.2/0.8        | Resin 10 B2         | 125                             | Xylene            | 16                | Cyclopentanone    | 38 | Methylal | 36 |
| Photosensitive member A-17 | A-1/A-2 7.2/0.8        | Resin 10 B2         | 125                             | Xylene            | 2                 | Cyclopentanone    | 43 | Methylal | 36 |
| Photosensitive member A-18 | A-1/A-2 7.2/0.8        | Resin 10 B2         | 125                             | Xylene            | 41                | Cyclopentanone    | 38 | Methylal | 36 |
| Photosensitive member A-19 | A-1/A-2 7.2/0.8        | Resin 10 B2         | 125                             | Xylene            | 16                | Cyclopentanone    | 50 | Methylal | 36 |

TABLE 2-continued

|                            | $\alpha$               | $\beta$                        | (( $\beta$ ) content/              | $\gamma$ | $\delta$      | Another solvent |               |          |               |
|----------------------------|------------------------|--------------------------------|------------------------------------|----------|---------------|-----------------|---------------|----------|---------------|
|                            | Parts by Compound mass | Parts by Resin by $\beta$ mass | ( $\alpha$ ) content) $\times$ 100 | Compound | Parts by mass | Compound        | Parts by mass | Compound | Parts by mass |
| Photosensitive member A-20 | A-1/A-2 7.2/ 0.8       | Resin 10 B2                    | 125                                | Xylene   | 2             | Cyclopentanone  | 46            | Methylal | 36            |
| Photosensitive member A-21 | A-1/A-2 7.2/ 0.8       | Resin 10 B2                    | 125                                | Xylene   | 21            | Cyclopentanone  | 23            | Methylal | 36            |
| Photosensitive member A-22 | A-1/A-2 7.2/ 0.8       | Resin 10 B2                    | 125                                | Xylene   | 16            | Cyclopentanone  | 23            | Methylal | 36            |
| Photosensitive member A-23 | A-1/A-2 7.2/ 0.8       | Resin 10 B2                    | 125                                | Xylene   | 13            | Cyclopentanone  | 23            | Methylal | 36            |
| Photosensitive member A-24 | A-1/A-2 7.2/ 0.8       | Resin 10 B2                    | 125                                | Xylene   | 8             | Cyclopentanone  | 23            | Methylal | 36            |
| Photosensitive member A-25 | A-1/A-2 7.2/ 0.8       | Resin 10 B2                    | 125                                | Xylene   | 1             | Cyclopentanone  | 40            | Methylal | 36            |
| Photosensitive member A-26 | A-1/A-2 7.2/ 0.8       | Resin 10 B2                    | 125                                | Xylene   | 21            | Cyclopentanone  | 33            | Methylal | 36            |
| Photosensitive member A-27 | A-1/A-2 7.2/ 0.8       | Resin 10 B2                    | 125                                | Xylene   | 16            | Cyclopentanone  | 33            | Methylal | 36            |
| Photosensitive member A-28 | A-1/A-2 7.2/ 0.8       | Resin 10 B2                    | 125                                | Xylene   | 13            | Cyclopentanone  | 33            | Methylal | 36            |
| Photosensitive member A-29 | A-1/A-2 7.2/ 0.8       | Resin 10 B2                    | 125                                | Xylene   | 8             | Cyclopentanone  | 33            | Methylal | 36            |
| Photosensitive member A-30 | A-1/A-2 7.2/ 0.8       | Resin 10 B2                    | 125                                | Xylene   | 1             | Cyclopentanone  | 45            | Methylal | 36            |
| Photosensitive member A-31 | A-1/A-2 7.2/ 0.8       | Resin 10/ B2/ 0.18             | 127.5                              | Xylene   | 16            | Cyclopentanone  | 28            | Methylal | 36            |
|                            |                        | Resin A3                       |                                    |          |               |                 |               |          |               |
| Photosensitive member A-32 | A-1/A-2 7.2/ 0.8       | Resin 10/ B2/ 0.2              | 127.5                              | Xylene   | 16            | Cyclopentanone  | 28            | Methylal | 36            |
|                            |                        | Resin C1                       |                                    |          |               |                 |               |          |               |
| Photosensitive member A-33 | A-1/A-2 7.2/ 0.8       | Resin 10/ B2/ 0.18             | 127.5                              | Xylene   | 16            | Cyclopentanone  | 28            | Methylal | 36            |
|                            |                        | Resin A3                       |                                    |          |               |                 |               |          |               |
| Photosensitive member A-34 | A-1/A-2 7.2/ 0.8       | Resin 10/ B2/ 0.2              | 127.5                              | Xylene   | 16            | Cyclopentanone  | 28            | Methylal | 36            |
|                            |                        | Resin C1                       |                                    |          |               |                 |               |          |               |
| Photosensitive member A-35 | A-1/A-2 7.2/ 0.8       | Resin 9.5/ B1/ 0.5/            | 126.25                             | Xylene   | 16            | Cyclopentanone  | 28            | Methylal | 36            |
|                            |                        | Resin 0.1                      |                                    |          |               |                 |               |          |               |
|                            |                        | A2/ Resin C1                   |                                    |          |               |                 |               |          |               |

TABLE 3

|                            | Drying temperature [° C.] | Drying time [min] | CTL thickness [μm] | $\gamma$ Content [%] | $\delta$ Content [%] | Percentage of $\gamma$ content to $\delta$ content |
|----------------------------|---------------------------|-------------------|--------------------|----------------------|----------------------|----------------------------------------------------|
| Photosensitive member A-1  | 120                       | 60                | 30                 | 1.20                 | 0.11                 | 1091                                               |
| Photosensitive member A-2  | 120                       | 60                | 30                 | 1.40                 | 0.12                 | 1167                                               |
| Photosensitive member A-3  | 120                       | 60                | 30                 | 0.95                 | 0.14                 | 667                                                |
| Photosensitive member A-4  | 120                       | 60                | 30                 | 1.48                 | 0.15                 | 987                                                |
| Photosensitive member A-5  | 120                       | 60                | 30                 | 0.92                 | 0.40                 | 230                                                |
| Photosensitive member A-6  | 120                       | 60                | 30                 | 1.42                 | 0.38                 | 375                                                |
| Photosensitive member A-7  | 120                       | 60                | 30                 | 1.98                 | 0.01                 | 20900                                              |
| Photosensitive member A-8  | 125                       | 60                | 30                 | 1.50                 | 0.01                 | 15833                                              |
| Photosensitive member A-9  | 125                       | 60                | 30                 | 0.95                 | 0.01                 | 10000                                              |
| Photosensitive member A-10 | 125                       | 60                | 30                 | 0.81                 | 0.01                 | 8550                                               |
| Photosensitive member A-11 | 130                       | 120               | 30                 | 0.01                 | 0.01                 | 100                                                |
| Photosensitive member A-12 | 120                       | 60                | 30                 | 2.00                 | 0.05                 | 4222                                               |
| Photosensitive member A-13 | 125                       | 60                | 30                 | 0.47                 | 0.05                 | 1000                                               |
| Photosensitive member A-14 | 120                       | 60                | 30                 | 0.01                 | 0.05                 | 20                                                 |
| Photosensitive member A-15 | 120                       | 60                | 30                 | 1.97                 | 0.15                 | 1313                                               |
| Photosensitive member A-16 | 125                       | 60                | 30                 | 0.40                 | 0.18                 | 222                                                |
| Photosensitive member A-17 | 120                       | 60                | 30                 | 0.01                 | 0.14                 | 7                                                  |
| Photosensitive member A-18 | 120                       | 60                | 30                 | 1.95                 | 0.38                 | 515                                                |
| Photosensitive member A-19 | 125                       | 60                | 30                 | 0.47                 | 0.42                 | 113                                                |

TABLE 3-continued

|                            | Drying temperature<br>[° C.] | Drying time<br>[min] | CTL thickness<br>[μm] | γ Content<br>[%] | δ Content<br>[%] | Percentage of γ content to δ content |
|----------------------------|------------------------------|----------------------|-----------------------|------------------|------------------|--------------------------------------|
| Photosensitive member A-20 | 120                          | 60                   | 30                    | 0.01             | 0.46             | 2                                    |
| Photosensitive member A-21 | 115                          | 60                   | 30                    | 1.79             | 0.79             | 227                                  |
| Photosensitive member A-22 | 115                          | 60                   | 30                    | 1.40             | 0.71             | 197                                  |
| Photosensitive member A-23 | 115                          | 60                   | 30                    | 0.95             | 0.75             | 126                                  |
| Photosensitive member A-24 | 115                          | 60                   | 30                    | 0.47             | 0.70             | 68                                   |
| Photosensitive member A-25 | 115                          | 60                   | 30                    | 0.01             | 0.74             | 1                                    |
| Photosensitive member A-26 | 115                          | 60                   | 30                    | 1.92             | 1.18             | 162                                  |
| Photosensitive member A-27 | 115                          | 60                   | 30                    | 1.42             | 1.20             | 118                                  |
| Photosensitive member A-28 | 115                          | 60                   | 30                    | 0.95             | 1.15             | 82                                   |
| Photosensitive member A-29 | 115                          | 60                   | 30                    | 0.47             | 1.16             | 41                                   |
| Photosensitive member A-30 | 115                          | 60                   | 30                    | 0.01             | 1.18             | 1                                    |
| Photosensitive member A-31 | 120                          | 60                   | 30                    | 1.11             | 0.10             | 1110                                 |
| Photosensitive member A-32 | 120                          | 60                   | 30                    | 1.16             | 0.07             | 1657                                 |
| Photosensitive member A-33 | 120                          | 60                   | 30                    | 1.01             | 0.12             | 842                                  |
| Photosensitive member A-34 | 120                          | 60                   | 30                    | 1.05             | 0.30             | 350                                  |
| Photosensitive member A-35 | 120                          | 60                   | 30                    | 1.31             | 0.23             | 570                                  |

TABLE 4

|                             | $\alpha$                     | $\beta$          | $((\beta))$<br>content/                                         | $\gamma$                | $\delta$                | Another solvent                 |                                 |             |
|-----------------------------|------------------------------|------------------|-----------------------------------------------------------------|-------------------------|-------------------------|---------------------------------|---------------------------------|-------------|
|                             | Parts<br>by<br>Compound mass | Resin<br>$\beta$ | Parts<br>by<br>mass<br>( $\alpha$ )<br>content) $\times$<br>100 | Parts<br>by<br>Compound | Parts<br>by<br>Compound | Parts<br>by<br>mass<br>Compound | Parts<br>by<br>mass<br>Compound |             |
| Photosensitive member A-101 | A-1/A-2 7.2/<br>0.8          | Resin B2         | 10                                                              | 125                     | Xylene                  | 16                              | Cyclopentanone 28               | Methylal 36 |
| Photosensitive member A-102 | A-1/A-2 7.2/<br>0.8          | Resin B2         | 10                                                              | 125                     | Xylene                  | 46                              | Cyclopentanone 0                | Methylal 36 |
| Photosensitive member A-103 | A-1/A-2 7.2/<br>0.8          | Resin B2         | 10                                                              | 125                     | Xylene                  | 46                              | Cyclopentanone 0                | Methylal 36 |
| Photosensitive member A-104 | A-1/A-2 7.2/<br>0.8          | Resin B2         | 10                                                              | 125                     | Xylene                  | 46                              | Cyclopentanone 0                | Methylal 36 |
| Photosensitive member A-105 | A-1/A-2 7.2/<br>0.8          | Resin B2         | 10                                                              | 125                     | Xylene                  | 0                               | Cyclopentanone 46               | Methylal 36 |
| Photosensitive member A-106 | A-1/A-2 7.2/<br>0.8          | Resin B2         | 10                                                              | 125                     | Xylene                  | 0                               | Cyclopentanone 46               | Methylal 36 |
| Photosensitive member A-107 | A-1/A-2 7.2/<br>0.8          | Resin B2         | 10                                                              | 125                     | Xylene                  | 21                              | Cyclopentanone 23               | Methylal 36 |
| Photosensitive member A-108 | A-1/A-2 7.2/<br>0.8          | Resin B2         | 10                                                              | 125                     | Xylene                  | 21                              | Cyclopentanone 35               | Methylal 36 |
| Photosensitive member A-109 | A-1/A-2 7.2/<br>0.8          | Resin B2         | 10                                                              | 125                     | Xylene                  | 15                              | Cyclopentanone 35               | Methylal 36 |
| Photosensitive member A-110 | A-1/A-2 7.2/<br>0.8          | Resin B2         | 10                                                              | 125                     | Xylene                  | 21                              | Cyclopentanone 35               | Methylal 36 |

TABLE 5

|                             | Drying temperature<br>[° C.] | Drying time<br>[min] | CTL thickness<br>[μm] | γ Content<br>[%] | δ Content<br>[%] | Percentage of γ content to δ content |
|-----------------------------|------------------------------|----------------------|-----------------------|------------------|------------------|--------------------------------------|
| Photosensitive member A-101 | 130                          | 130                  | 30                    | 0                | 0                | —                                    |
| Photosensitive member A-102 | 125                          | 60                   | 30                    | 0.88             | 0                | —                                    |
| Photosensitive member A-103 | 120                          | 90                   | 30                    | 1.81             | 0                | —                                    |
| Photosensitive member A-104 | 120                          | 60                   | 30                    | 2.43             | 0                | —                                    |
| Photosensitive member A-105 | 125                          | 60                   | 30                    | 0                | 0.16             | 0                                    |
| Photosensitive member A-106 | 120                          | 60                   | 30                    | 0                | 1.5              | 0                                    |
| Photosensitive member A-107 | 115                          | 45                   | 30                    | 2.55             | 0.14             | 1821                                 |
| Photosensitive member A-108 | 115                          | 60                   | 30                    | 2.68             | 1.61             | 166                                  |
| Photosensitive member A-109 | 115                          | 60                   | 30                    | 0.92             | 1.53             | 60                                   |
| Photosensitive member A-110 | 115                          | 60                   | 30                    | 2.25             | 1.55             | 145                                  |

TABLE 6

|                            | $\alpha$               | $\beta$       | (( $\beta$ ) content/ | $\gamma$                           | $\delta$          | Another solvent |                   |    |          |    |
|----------------------------|------------------------|---------------|-----------------------|------------------------------------|-------------------|-----------------|-------------------|----|----------|----|
|                            | Parts by Compound mass | Resin $\beta$ | Parts by mass         | ( $\alpha$ ) content) $\times$ 100 | Parts by Compound | Parts by mass   | Parts by Compound |    |          |    |
| Photosensitive member B-1  | A-1/A-2 5.4/0.6        | Resin B2      | 12                    | 200                                | Xylene            | 16              | Cyclopentanone    | 28 | Methylal | 36 |
| Photosensitive member B-2  | A-1/A-2 5.4/0.6        | Resin B2      | 12                    | 200                                | Xylene            | 21              | Cyclopentanone    | 23 | Methylal | 36 |
| Photosensitive member B-3  | A-1/A-2 5.4/0.6        | Resin B2      | 12                    | 200                                | Xylene            | 16              | Cyclopentanone    | 30 | Methylal | 36 |
| Photosensitive member B-4  | A-1/A-2 5.4/0.6        | Resin B2      | 12                    | 200                                | Xylene            | 21              | Cyclopentanone    | 25 | Methylal | 36 |
| Photosensitive member B-5  | A-1/A-2 5.4/0.6        | Resin B2      | 12                    | 200                                | Xylene            | 8               | Cyclopentanone    | 38 | Methylal | 36 |
| Photosensitive member B-6  | A-1/A-2 5.4/0.6        | Resin B2      | 12                    | 200                                | Xylene            | 14              | Cyclopentanone    | 38 | Methylal | 36 |
| Photosensitive member B-7  | A-1/A-2 5.4/0.6        | Resin B2      | 12                    | 200                                | Xylene            | 41              | Cyclopentanone    | 5  | Methylal | 36 |
| Photosensitive member B-8  | A-1/A-2 5.4/0.6        | Resin B2      | 12                    | 200                                | Xylene            | 41              | Cyclopentanone    | 5  | Methylal | 36 |
| Photosensitive member B-9  | A-1/A-2 5.4/0.6        | Resin B2      | 12                    | 200                                | Xylene            | 33              | Cyclopentanone    | 13 | Methylal | 36 |
| Photosensitive member B-10 | A-1/A-2 5.4/0.6        | Resin B2      | 12                    | 200                                | Xylene            | 21              | Cyclopentanone    | 23 | Methylal | 36 |
| Photosensitive member B-11 | A-1/A-2 5.4/0.6        | Resin B2      | 12                    | 200                                | Xylene            | 16              | Cyclopentanone    | 28 | Methylal | 36 |
| Photosensitive member B-12 | A-1/A-2 5.4/0.6        | Resin B2      | 12                    | 200                                | Xylene            | 41              | Cyclopentanone    | 20 | Methylal | 36 |
| Photosensitive member B-13 | A-1/A-2 5.4/0.6        | Resin B2      | 12                    | 200                                | Xylene            | 16              | Cyclopentanone    | 30 | Methylal | 36 |
| Photosensitive member B-14 | A-1/A-2 5.4/0.6        | Resin B2      | 12                    | 200                                | Xylene            | 2               | Cyclopentanone    | 40 | Methylal | 36 |
| Photosensitive member B-15 | A-1/A-2 5.4/0.6        | Resin B2      | 12                    | 200                                | Xylene            | 41              | Cyclopentanone    | 35 | Methylal | 36 |
| Photosensitive member B-16 | A-1/A-2 5.4/0.6        | Resin B2      | 12                    | 200                                | Xylene            | 16              | Cyclopentanone    | 38 | Methylal | 36 |
| Photosensitive member B-17 | A-1/A-2 5.4/0.6        | Resin B2      | 12                    | 200                                | Xylene            | 2               | Cyclopentanone    | 43 | Methylal | 36 |
| Photosensitive member B-18 | A-1/A-2 5.4/0.6        | Resin B2      | 12                    | 200                                | Xylene            | 41              | Cyclopentanone    | 38 | Methylal | 36 |
| Photosensitive member B-19 | A-1/A-2 5.4/0.6        | Resin B2      | 12                    | 200                                | Xylene            | 16              | Cyclopentanone    | 50 | Methylal | 36 |
| Photosensitive member B-20 | A-1/A-2 5.4/0.6        | Resin B2      | 12                    | 200                                | Xylene            | 2               | Cyclopentanone    | 46 | Methylal | 36 |
| Photosensitive member B-21 | A-1/A-2 5.4/0.6        | Resin B2      | 12                    | 200                                | Xylene            | 21              | Cyclopentanone    | 23 | Methylal | 36 |
| Photosensitive member B-22 | A-1/A-2 5.4/0.6        | Resin B2      | 12                    | 200                                | Xylene            | 16              | Cyclopentanone    | 23 | Methylal | 36 |
| Photosensitive member B-23 | A-1/A-2 5.4/0.6        | Resin B2      | 12                    | 200                                | Xylene            | 13              | Cyclopentanone    | 23 | Methylal | 36 |
| Photosensitive member B-24 | A-1/A-2 5.4/0.6        | Resin B2      | 12                    | 200                                | Xylene            | 8               | Cyclopentanone    | 23 | Methylal | 36 |
| Photosensitive member B-25 | A-1/A-2 5.4/0.6        | Resin B2      | 12                    | 200                                | Xylene            | 1               | Cyclopentanone    | 40 | Methylal | 36 |
| Photosensitive member B-26 | A-1/A-2 5.4/0.6        | Resin B2      | 12                    | 200                                | Xylene            | 21              | Cyclopentanone    | 33 | Methylal | 36 |
| Photosensitive member B-27 | A-1/A-2 5.4/0.6        | Resin B2      | 12                    | 200                                | Xylene            | 16              | Cyclopentanone    | 33 | Methylal | 36 |
| Photosensitive member B-28 | A-1/A-2 5.4/0.6        | Resin B2      | 12                    | 200                                | Xylene            | 13              | Cyclopentanone    | 33 | Methylal | 36 |
| Photosensitive member B-29 | A-1/A-2 5.4/0.6        | Resin B2      | 12                    | 200                                | Xylene            | 8               | Cyclopentanone    | 33 | Methylal | 36 |
| Photosensitive member B-30 | A-1/A-2 5.4/0.6        | Resin B2      | 12                    | 200                                | Xylene            | 1               | Cyclopentanone    | 45 | Methylal | 36 |

TABLE 7

|                           | Drying temperature [°C.] | Drying time [min] | CTL thickness [μm] | $\gamma$ Content [%] | $\delta$ Content [%] | Percentage of $\gamma$ content to $\delta$ content |
|---------------------------|--------------------------|-------------------|--------------------|----------------------|----------------------|----------------------------------------------------|
| Photosensitive member B-1 | 120                      | 60                | 30                 | 1.01                 | 0.15                 | 673                                                |
| Photosensitive member B-2 | 120                      | 60                | 30                 | 1.32                 | 0.10                 | 1320                                               |

TABLE 7-continued

|                            | Drying temperature [° C.] | Drying time [min] | CTL thickness [μm] | γ Content [%] | δ Content [%] | Percentage of γ content to δ content |
|----------------------------|---------------------------|-------------------|--------------------|---------------|---------------|--------------------------------------|
| Photosensitive member B-3  | 120                       | 60                | 30                 | 0.85          | 0.16          | 531                                  |
| Photosensitive member B-4  | 120                       | 60                | 30                 | 1.42          | 0.33          | 430                                  |
| Photosensitive member B-5  | 120                       | 60                | 30                 | 0.98          | 0.35          | 280                                  |
| Photosensitive member B-6  | 120                       | 60                | 30                 | 1.41          | 0.49          | 288                                  |
| Photosensitive member B-7  | 120                       | 60                | 30                 | 1.88          | 0.01          | 19844                                |
| Photosensitive member B-8  | 125                       | 60                | 30                 | 1.43          | 0.01          | 15094                                |
| Photosensitive member B-9  | 125                       | 60                | 30                 | 1.12          | 0.01          | 11822                                |
| Photosensitive member B-10 | 125                       | 60                | 30                 | 0.73          | 0.01          | 7706                                 |
| Photosensitive member B-11 | 130                       | 120               | 30                 | 0.01          | 0.01          | 100                                  |
| Photosensitive member B-12 | 120                       | 60                | 30                 | 1.91          | 0.04          | 4775                                 |
| Photosensitive member B-13 | 125                       | 60                | 30                 | 0.59          | 0.05          | 1246                                 |
| Photosensitive member B-14 | 120                       | 60                | 30                 | 0.01          | 0.05          | 20                                   |
| Photosensitive member B-15 | 120                       | 60                | 30                 | 1.96          | 0.18          | 1089                                 |
| Photosensitive member B-16 | 125                       | 60                | 30                 | 0.31          | 0.12          | 258                                  |
| Photosensitive member B-17 | 120                       | 60                | 30                 | 0.01          | 0.13          | 7                                    |
| Photosensitive member B-18 | 120                       | 60                | 30                 | 1.92          | 0.38          | 505                                  |
| Photosensitive member B-19 | 125                       | 60                | 30                 | 0.53          | 0.48          | 110                                  |
| Photosensitive member B-20 | 120                       | 60                | 30                 | 0.01          | 0.45          | 2                                    |
| Photosensitive member B-21 | 115                       | 60                | 30                 | 1.88          | 0.71          | 265                                  |
| Photosensitive member B-22 | 115                       | 60                | 30                 | 1.49          | 0.79          | 189                                  |
| Photosensitive member B-23 | 115                       | 60                | 30                 | 1.01          | 0.76          | 133                                  |
| Photosensitive member B-24 | 115                       | 60                | 30                 | 0.50          | 0.72          | 69                                   |
| Photosensitive member B-25 | 115                       | 60                | 30                 | 0.01          | 0.78          | 1                                    |
| Photosensitive member B-26 | 115                       | 60                | 30                 | 1.89          | 1.14          | 166                                  |
| Photosensitive member B-27 | 115                       | 60                | 30                 | 1.46          | 1.16          | 126                                  |
| Photosensitive member B-28 | 115                       | 60                | 30                 | 1.12          | 1.16          | 97                                   |
| Photosensitive member B-29 | 115                       | 60                | 30                 | 0.49          | 1.19          | 41                                   |
| Photosensitive member B-30 | 115                       | 60                | 30                 | 0.01          | 1.10          | 1                                    |

TABLE 8

|                             | α       | β           | ((β)) content/            |                        | γ                        |          | δ                |                | Another solvent  |          |    |
|-----------------------------|---------|-------------|---------------------------|------------------------|--------------------------|----------|------------------|----------------|------------------|----------|----|
|                             |         |             | Parts by<br>Compound mass | Parts by<br>Resin mass | (α)<br>content) ×<br>100 | Compound | Parts by<br>mass | Compound       | Parts by<br>mass | Compound |    |
| Photosensitive member B-101 | A-1/A-2 | 5.4/<br>0.6 | Resin<br>B2               | 12                     | 200                      | Xylene   | 16               | Cyclopentanone | 28               | Methylal | 36 |
| Photosensitive member B-102 | A-1/A-2 | 5.4/<br>0.6 | Resin<br>B2               | 12                     | 200                      | Xylene   | 46               | Cyclopentanone | 0                | Methylal | 36 |
| Photosensitive member B-103 | A-1/A-2 | 5.4/<br>0.6 | Resin<br>B2               | 12                     | 200                      | Xylene   | 46               | Cyclopentanone | 0                | Methylal | 36 |
| Photosensitive member B-104 | A-1/A-2 | 5.4/<br>0.6 | Resin<br>B2               | 12                     | 200                      | Xylene   | 46               | Cyclopentanone | 0                | Methylal | 36 |
| Photosensitive member B-105 | A-1/A-2 | 5.4/<br>0.6 | Resin<br>B2               | 12                     | 200                      | Xylene   | 0                | Cyclopentanone | 46               | Methylal | 36 |
| Photosensitive member B-106 | A-1/A-2 | 5.4/<br>0.6 | Resin<br>B2               | 12                     | 200                      | Xylene   | 0                | Cyclopentanone | 46               | Methylal | 36 |
| Photosensitive member B-107 | A-1/A-2 | 5.4/<br>0.6 | Resin<br>B2               | 12                     | 200                      | Xylene   | 21               | Cyclopentanone | 23               | Methylal | 36 |
| Photosensitive member B-108 | A-1/A-2 | 5.4/<br>0.6 | Resin<br>B2               | 12                     | 200                      | Xylene   | 21               | Cyclopentanone | 35               | Methylal | 36 |
| Photosensitive member B-109 | A-1/A-2 | 5.4/<br>0.6 | Resin<br>B2               | 12                     | 200                      | Xylene   | 15               | Cyclopentanone | 35               | Methylal | 36 |
| Photosensitive member B-110 | A-1/A-2 | 5.4/<br>0.6 | Resin<br>B2               | 12                     | 200                      | Xylene   | 21               | Cyclopentanone | 35               | Methylal | 36 |

TABLE 9

|                             | Drying temperature [° C.] | Drying time [min] | CTL thickness [μm] | γ Content [%] | δ Content [%] | Percentage of γ content to δ content |
|-----------------------------|---------------------------|-------------------|--------------------|---------------|---------------|--------------------------------------|
| Photosensitive member B-101 | 130                       | 130               | 30                 | 0             | 0             | —                                    |
| Photosensitive member B-102 | 125                       | 60                | 30                 | 0.79          | 0             | —                                    |

TABLE 9-continued

|                             | Drying temperature<br>[° C.] | Drying time<br>[min] | CTL thickness<br>[μm] | γ Content<br>[%] | δ Content<br>[%] | Percentage of γ content to δ content |
|-----------------------------|------------------------------|----------------------|-----------------------|------------------|------------------|--------------------------------------|
| Photosensitive member B-103 | 120                          | 90                   | 30                    | 1.91             | 0                | —                                    |
| Photosensitive member B-104 | 120                          | 60                   | 30                    | 2.6              | 0                | —                                    |
| Photosensitive member B-105 | 125                          | 60                   | 30                    | 0                | 0.14             | 0                                    |
| Photosensitive member B-106 | 120                          | 60                   | 30                    | 0                | 1.62             | 0                                    |
| Photosensitive member B-107 | 115                          | 45                   | 30                    | 2.13             | 0.16             | 1331                                 |
| Photosensitive member B-108 | 115                          | 60                   | 30                    | 2.54             | 1.65             | 154                                  |
| Photosensitive member B-109 | 115                          | 60                   | 30                    | 0.82             | 1.47             | 56                                   |
| Photosensitive member B-110 | 115                          | 60                   | 30                    | 2.3              | 1.61             | 143                                  |

TABLE 10

|                            | α<br>Compound | β<br>Parts by mass | ((β) content/<br>(α) content) × 100 |                  | γ<br>Compound | δ<br>Parts by mass | Another solvent  |                  |    |          |    |
|----------------------------|---------------|--------------------|-------------------------------------|------------------|---------------|--------------------|------------------|------------------|----|----------|----|
|                            |               |                    | Parts by<br>Resin<br>β              | Parts by<br>mass |               |                    | Parts by<br>mass | Parts by<br>mass |    |          |    |
|                            |               |                    | Compound                            | mass             | Compound      | mass               | Compound         | mass             |    |          |    |
| Photosensitive member C-1  | A-1/A-2       | 11/1               | Resin B2                            | 6                | 50            | Xylene             | 16               | Cyclopentanone   | 28 | Methylal | 36 |
| Photosensitive member C-2  | A-1/A-2       | 11/1               | Resin B2                            | 6                | 50            | Xylene             | 21               | Cyclopentanone   | 23 | Methylal | 36 |
| Photosensitive member C-3  | A-1/A-2       | 11/1               | Resin B2                            | 6                | 50            | Xylene             | 16               | Cyclopentanone   | 30 | Methylal | 36 |
| Photosensitive member C-4  | A-1/A-2       | 11/1               | Resin B2                            | 6                | 50            | Xylene             | 21               | Cyclopentanone   | 25 | Methylal | 36 |
| Photosensitive member C-5  | A-1/A-2       | 11/1               | Resin B2                            | 6                | 50            | Xylene             | 8                | Cyclopentanone   | 38 | Methylal | 36 |
| Photosensitive member C-6  | A-1/A-2       | 11/1               | Resin B2                            | 6                | 50            | Xylene             | 14               | Cyclopentanone   | 38 | Methylal | 36 |
| Photosensitive member C-7  | A-1/A-2       | 11/1               | Resin B2                            | 6                | 50            | Xylene             | 41               | Cyclopentanone   | 5  | Methylal | 36 |
| Photosensitive member C-8  | A-1/A-2       | 11/1               | Resin B2                            | 6                | 50            | Xylene             | 41               | Cyclopentanone   | 5  | Methylal | 36 |
| Photosensitive member C-9  | A-1/A-2       | 11/1               | Resin B2                            | 6                | 50            | Xylene             | 33               | Cyclopentanone   | 13 | Methylal | 36 |
| Photosensitive member C-10 | A-1/A-2       | 11/1               | Resin B2                            | 6                | 50            | Xylene             | 21               | Cyclopentanone   | 23 | Methylal | 36 |
| Photosensitive member C-11 | A-1/A-2       | 11/1               | Resin B2                            | 6                | 50            | Xylene             | 16               | Cyclopentanone   | 28 | Methylal | 36 |
| Photosensitive member C-12 | A-1/A-2       | 11/1               | Resin B2                            | 6                | 50            | Xylene             | 41               | Cyclopentanone   | 20 | Methylal | 36 |
| Photosensitive member C-13 | A-1/A-2       | 11/1               | Resin B2                            | 6                | 50            | Xylene             | 16               | Cyclopentanone   | 30 | Methylal | 36 |
| Photosensitive member C-14 | A-1/A-2       | 11/1               | Resin B2                            | 6                | 50            | Xylene             | 2                | Cyclopentanone   | 40 | Methylal | 36 |
| Photosensitive member C-15 | A-1/A-2       | 11/1               | Resin B2                            | 6                | 50            | Xylene             | 41               | Cyclopentanone   | 35 | Methylal | 36 |
| Photosensitive member C-16 | A-1/A-2       | 11/1               | Resin B2                            | 6                | 50            | Xylene             | 16               | Cyclopentanone   | 38 | Methylal | 36 |
| Photosensitive member C-17 | A-1/A-2       | 11/1               | Resin B2                            | 6                | 50            | Xylene             | 2                | Cyclopentanone   | 43 | Methylal | 36 |
| Photosensitive member C-18 | A-1/A-2       | 11/1               | Resin B2                            | 6                | 50            | Xylene             | 41               | Cyclopentanone   | 38 | Methylal | 36 |
| Photosensitive member C-19 | A-1/A-2       | 11/1               | Resin B2                            | 6                | 50            | Xylene             | 16               | Cyclopentanone   | 50 | Methylal | 36 |
| Photosensitive member C-20 | A-1/A-2       | 11/1               | Resin B2                            | 6                | 50            | Xylene             | 2                | Cyclopentanone   | 46 | Methylal | 36 |
| Photosensitive member C-21 | A-1/A-2       | 11/1               | Resin B2                            | 6                | 50            | Xylene             | 21               | Cyclopentanone   | 23 | Methylal | 36 |
| Photosensitive member C-22 | A-1/A-2       | 11/1               | Resin B2                            | 6                | 50            | Xylene             | 16               | Cyclopentanone   | 23 | Methylal | 36 |
| Photosensitive member C-23 | A-1/A-2       | 11/1               | Resin B2                            | 6                | 50            | Xylene             | 13               | Cyclopentanone   | 23 | Methylal | 36 |
| Photosensitive member C-24 | A-1/A-2       | 11/1               | Resin B2                            | 6                | 50            | Xylene             | 8                | Cyclopentanone   | 23 | Methylal | 36 |
| Photosensitive member C-25 | A-1/A-2       | 11/1               | Resin B2                            | 6                | 50            | Xylene             | 1                | Cyclopentanone   | 40 | Methylal | 36 |
| Photosensitive member C-26 | A-1/A-2       | 11/1               | Resin B2                            | 6                | 50            | Xylene             | 21               | Cyclopentanone   | 33 | Methylal | 36 |
| Photosensitive member C-27 | A-1/A-2       | 11/1               | Resin B2                            | 6                | 50            | Xylene             | 16               | Cyclopentanone   | 33 | Methylal | 36 |

TABLE 10-continued

|                            | $\alpha$ | $\beta$       | (( $\beta$ ) content/ |               | $\gamma$ | $\delta$ | Another solvent |                |               |          |    |
|----------------------------|----------|---------------|-----------------------|---------------|----------|----------|-----------------|----------------|---------------|----------|----|
|                            |          |               | Parts by mass         | Parts by mass |          |          | Parts by mass   | Parts by mass  | Parts by mass |          |    |
|                            | Compound | Resin $\beta$ | Compound              | Compound      | Compound | Compound | Compound        | Compound       | Compound      |          |    |
| Photosensitive member C-28 | A-1/A-2  | 11/1          | Resin B2              | 6             | 50       | Xylene   | 13              | Cyclopentanone | 33            | Methylal | 36 |
| Photosensitive member C-29 | A-1/A-2  | 11/1          | Resin B2              | 6             | 50       | Xylene   | 8               | Cyclopentanone | 33            | Methylal | 36 |
| Photosensitive member C-30 | A-1/A-2  | 11/1          | Resin B2              | 6             | 50       | Xylene   | 1               | Cyclopentanone | 45            | Methylal | 36 |

TABLE 11

|                            | Drying temperature [° C.] | Drying time [min] | CTL thickness [μm] | $\gamma$ Content [%] | $\delta$ Content [%] | Percentage of $\gamma$ content to $\delta$ content |
|----------------------------|---------------------------|-------------------|--------------------|----------------------|----------------------|----------------------------------------------------|
| Photosensitive member C-1  | 120                       | 60                | 30                 | 1.10                 | 0.13                 | 846                                                |
| Photosensitive member C-2  | 120                       | 60                | 30                 | 1.32                 | 0.11                 | 1200                                               |
| Photosensitive member C-3  | 120                       | 60                | 30                 | 1.01                 | 0.15                 | 673                                                |
| Photosensitive member C-4  | 120                       | 60                | 30                 | 1.45                 | 0.12                 | 1208                                               |
| Photosensitive member C-5  | 120                       | 60                | 30                 | 0.90                 | 0.38                 | 237                                                |
| Photosensitive member C-6  | 120                       | 60                | 30                 | 1.49                 | 0.32                 | 466                                                |
| Photosensitive member C-7  | 120                       | 60                | 30                 | 1.91                 | 0.01                 | 20161                                              |
| Photosensitive member C-8  | 125                       | 60                | 30                 | 1.32                 | 0.01                 | 13933                                              |
| Photosensitive member C-9  | 125                       | 60                | 30                 | 1.12                 | 0.01                 | 11822                                              |
| Photosensitive member C-10 | 125                       | 60                | 30                 | 0.73                 | 0.01                 | 7706                                               |
| Photosensitive member C-11 | 130                       | 120               | 30                 | 0.01                 | 0.01                 | 100                                                |
| Photosensitive member C-12 | 120                       | 60                | 30                 | 1.88                 | 0.04                 | 4700                                               |
| Photosensitive member C-13 | 125                       | 60                | 30                 | 0.50                 | 0.05                 | 1000                                               |
| Photosensitive member C-14 | 120                       | 60                | 30                 | 0.01                 | 0.04                 | 24                                                 |
| Photosensitive member C-15 | 120                       | 60                | 30                 | 1.91                 | 0.18                 | 1061                                               |
| Photosensitive member C-16 | 125                       | 60                | 30                 | 0.35                 | 0.15                 | 233                                                |
| Photosensitive member C-17 | 120                       | 60                | 30                 | 0.01                 | 0.12                 | 8                                                  |
| Photosensitive member C-18 | 120                       | 60                | 30                 | 1.80                 | 0.44                 | 409                                                |
| Photosensitive member C-19 | 125                       | 60                | 30                 | 0.53                 | 0.48                 | 110                                                |
| Photosensitive member C-20 | 120                       | 60                | 30                 | 0.01                 | 0.32                 | 3                                                  |
| Photosensitive member C-21 | 115                       | 60                | 30                 | 1.99                 | 0.74                 | 269                                                |
| Photosensitive member C-22 | 115                       | 60                | 30                 | 1.49                 | 0.79                 | 189                                                |
| Photosensitive member C-23 | 115                       | 60                | 30                 | 0.82                 | 0.71                 | 115                                                |
| Photosensitive member C-24 | 115                       | 60                | 30                 | 0.52                 | 0.76                 | 68                                                 |
| Photosensitive member C-25 | 115                       | 60                | 30                 | 0.01                 | 0.79                 | 1                                                  |
| Photosensitive member C-26 | 115                       | 60                | 30                 | 1.84                 | 1.10                 | 167                                                |
| Photosensitive member C-27 | 115                       | 60                | 30                 | 1.44                 | 1.24                 | 116                                                |
| Photosensitive member C-28 | 115                       | 60                | 30                 | 1.10                 | 1.18                 | 93                                                 |
| Photosensitive member C-29 | 115                       | 60                | 30                 | 0.42                 | 1.09                 | 39                                                 |
| Photosensitive member C-30 | 115                       | 60                | 30                 | 0.01                 | 1.16                 | 1                                                  |

TABLE 12

|                             | $\alpha$ | $\beta$       | (( $\beta$ ) content/ |               | $\gamma$ | $\delta$ | Another solvent |                |               |          |    |
|-----------------------------|----------|---------------|-----------------------|---------------|----------|----------|-----------------|----------------|---------------|----------|----|
|                             |          |               | Parts by mass         | Parts by mass |          |          | Parts by mass   | Parts by mass  | Parts by mass |          |    |
|                             | Compound | Resin $\beta$ | Compound              | Compound      | Compound | Compound | Compound        | Compound       | Compound      |          |    |
| Photosensitive member C-101 | A-1/A-2  | 11/1          | Resin B2              | 6             | 50       | Xylene   | 16              | Cyclopentanone | 28            | Methylal | 36 |
| Photosensitive member C-102 | A-1/A-2  | 11/1          | Resin B2              | 6             | 50       | Xylene   | 46              | Cyclopentanone | 0             | Methylal | 36 |
| Photosensitive member C-103 | A-1/A-2  | 11/1          | Resin B2              | 6             | 50       | Xylene   | 46              | Cyclopentanone | 0             | Methylal | 36 |
| Photosensitive member C-104 | A-1/A-2  | 11/1          | Resin B2              | 6             | 50       | Xylene   | 46              | Cyclopentanone | 0             | Methylal | 36 |
| Photosensitive member C-105 | A-1/A-2  | 11/1          | Resin B2              | 6             | 50       | Xylene   | 0               | Cyclopentanone | 46            | Methylal | 36 |
| Photosensitive member C-106 | A-1/A-2  | 11/1          | Resin B2              | 6             | 50       | Xylene   | 0               | Cyclopentanone | 46            | Methylal | 36 |
| Photosensitive member C-107 | A-1/A-2  | 11/1          | Resin B2              | 6             | 50       | Xylene   | 21              | Cyclopentanone | 23            | Methylal | 36 |

TABLE 12-continued

|                             | $\alpha$ | $\beta$ | (( $\beta$ ) content/ |               | $\gamma$ | $\delta$                   |               | Another solvent |               |          |    |
|-----------------------------|----------|---------|-----------------------|---------------|----------|----------------------------|---------------|-----------------|---------------|----------|----|
|                             |          |         | Parts by mass         | Parts by mass |          | ( $\alpha$ ) content × 100 | Parts by mass | Parts by mass   | Parts by mass |          |    |
|                             |          |         | Compound              | Resin $\beta$ |          | content × 100              | Compound      | Compound        | Compound      |          |    |
| Photosensitive member C-108 | A-1/A-2  | 11/1    | Resin B2              | 6             | 50       | Xylene                     | 21            | Cyclopentanone  | 35            | Methylal | 36 |
| Photosensitive member C-109 | A-1/A-2  | 11/1    | Resin B2              | 6             | 50       | Xylene                     | 15            | Cyclopentanone  | 35            | Methylal | 36 |
| Photosensitive member C-110 | A-1/A-2  | 11/1    | Resin B2              | 6             | 50       | Xylene                     | 21            | Cyclopentanone  | 35            | Methylal | 36 |

TABLE 13

|                             | Drying temperature [°C.] | Drying time [min] | CTL thickness [μm] | $\gamma$ Content [%] | $\delta$ Content [%] | Percentage of $\gamma$ content to $\delta$ content |
|-----------------------------|--------------------------|-------------------|--------------------|----------------------|----------------------|----------------------------------------------------|
| Photosensitive member C-101 | 130                      | 130               | 30                 | 0                    | 0                    | —                                                  |
| Photosensitive member C-102 | 125                      | 60                | 30                 | 0.93                 | 0                    | —                                                  |
| Photosensitive member C-103 | 120                      | 90                | 30                 | 1.9                  | 0                    | —                                                  |
| Photosensitive member C-104 | 120                      | 60                | 30                 | 2.21                 | 0                    | —                                                  |
| Photosensitive member C-105 | 125                      | 60                | 30                 | 0                    | 0.21                 | 0                                                  |
| Photosensitive member C-106 | 120                      | 60                | 30                 | 0                    | 1.33                 | 0                                                  |
| Photosensitive member C-107 | 115                      | 45                | 30                 | 2.61                 | 0.11                 | 2373                                               |
| Photosensitive member C-108 | 115                      | 60                | 30                 | 2.5                  | 1.58                 | 158                                                |
| Photosensitive member C-109 | 115                      | 60                | 30                 | 0.88                 | 1.6                  | 55                                                 |
| Photosensitive member C-110 | 115                      | 60                | 30                 | 2.3                  | 1.63                 | 141                                                |

TABLE 14

|                           | $\alpha$ | $\beta$ | (( $\beta$ ) content/ |               | $\gamma$ | $\delta$                   |               | Another solvent |               |          |    |
|---------------------------|----------|---------|-----------------------|---------------|----------|----------------------------|---------------|-----------------|---------------|----------|----|
|                           |          |         | Parts by mass         | Parts by mass |          | ( $\alpha$ ) content × 100 | Parts by mass | Parts by mass   | Parts by mass |          |    |
|                           |          |         | Compound              | Resin $\beta$ |          | content × 100              | Compound      | Compound        | Compound      |          |    |
| Photosensitive member D-1 | A-3      | 8       | Resin A1              | 10            | 125      | Xylene                     | 16            | Cyclopentanone  | 28            | Methylal | 36 |
| Photosensitive member D-2 | A-3      | 8       | Resin A1              | 10            | 125      | Xylene                     | 21            | Cyclopentanone  | 23            | Methylal | 36 |
| Photosensitive member D-3 | A-3      | 8       | Resin A1              | 10            | 125      | Xylene                     | 16            | Cyclopentanone  | 30            | Methylal | 36 |
| Photosensitive member D-4 | A-3      | 8       | Resin A1              | 10            | 125      | Xylene                     | 21            | Cyclopentanone  | 25            | Methylal | 36 |
| Photosensitive member D-5 | A-3      | 8       | Resin A1              | 10            | 125      | Xylene                     | 8             | Cyclopentanone  | 38            | Methylal | 36 |
| Photosensitive member D-6 | A-3      | 8       | Resin A1              | 10            | 125      | Xylene                     | 14            | Cyclopentanone  | 38            | Methylal | 36 |
| Photosensitive member D-7 | A-3      | 8       | Resin A1              | 10            | 125      | Xylene                     | 21            | Cyclopentanone  | 23            | Methylal | 36 |
| Photosensitive member D-8 | A-3      | 8       | Resin A1              | 10            | 125      | Xylene                     | 16            | Cyclopentanone  | 30            | Methylal | 36 |
| Photosensitive member D-9 | A-3      | 8       | Resin A1              | 10            | 125      | Xylene                     | 16            | Cyclopentanone  | 38            | Methylal | 36 |

TABLE 15

|                           | Drying temperature [°C.] | Drying time [min] | CTL thickness [μm] | $\gamma$ Content [%] | $\delta$ Content [%] | Percentage of $\gamma$ content to $\delta$ content |
|---------------------------|--------------------------|-------------------|--------------------|----------------------|----------------------|----------------------------------------------------|
| Photosensitive member D-1 | 120                      | 60                | 20                 | 0.85                 | 0.09                 | 944                                                |
| Photosensitive member D-2 | 120                      | 60                | 20                 | 1.31                 | 0.08                 | 1638                                               |
| Photosensitive member D-3 | 120                      | 60                | 20                 | 0.62                 | 0.12                 | 517                                                |
| Photosensitive member D-4 | 120                      | 60                | 20                 | 1.28                 | 0.13                 | 985                                                |
| Photosensitive member D-5 | 120                      | 60                | 20                 | 0.83                 | 0.38                 | 218                                                |
| Photosensitive member D-6 | 120                      | 60                | 20                 | 1.28                 | 0.29                 | 441                                                |
| Photosensitive member D-7 | 125                      | 60                | 20                 | 0.68                 | 0.01                 | 7178                                               |
| Photosensitive member D-8 | 125                      | 60                | 20                 | 0.42                 | 0.04                 | 1050                                               |
| Photosensitive member D-9 | 125                      | 45                | 20                 | 0.48                 | 0.12                 | 400                                                |

TABLE 16

| Compound                    | $\alpha$ | $\beta$    | (( $\beta$ ) content/ |               | $\gamma$                 | $\delta$      | Another solvent |                |
|-----------------------------|----------|------------|-----------------------|---------------|--------------------------|---------------|-----------------|----------------|
|                             |          |            | Parts by mass         | Parts by mass |                          |               | Parts by mass   | Parts by mass  |
|                             |          |            | Resin $\beta$         | Resin mass    | ( $\alpha$ ) content/100 | Parts by mass | Compound        | Compound       |
| Photosensitive member D-101 | A-3      | 8 Resin A1 | 10                    | 125           | Xylene                   | 16            | Cyclopentanone  | 28 Methylal 36 |
| Photosensitive member D-102 | A-3      | 8 Resin A1 | 10                    | 125           | Xylene                   | 46            | Cyclopentanone  | 0 Methylal 36  |
| Photosensitive member D-103 | A-3      | 8 Resin A1 | 10                    | 125           | Xylene                   | 46            | Cyclopentanone  | 0 Methylal 36  |
| Photosensitive member D-104 | A-3      | 8 Resin A1 | 10                    | 125           | Xylene                   | 0             | Cyclopentanone  | 46 Methylal 36 |
| Photosensitive member D-105 | A-3      | 8 Resin A1 | 10                    | 125           | Xylene                   | 0             | Cyclopentanone  | 46 Methylal 36 |
| Photosensitive member D-106 | A-3      | 8 Resin A1 | 10                    | 125           | Xylene                   | 21            | Cyclopentanone  | 23 Methylal 36 |
| Photosensitive member D-107 | A-3      | 8 Resin A1 | 10                    | 125           | Xylene                   | 21            | Cyclopentanone  | 35 Methylal 36 |
| Photosensitive member D-108 | A-3      | 8 Resin A1 | 10                    | 125           | Xylene                   | 15            | Cyclopentanone  | 35 Methylal 36 |
| Photosensitive member D-109 | A-3      | 8 Resin A1 | 10                    | 125           | Xylene                   | 21            | Cyclopentanone  | 35 Methylal 36 |

TABLE 17

|                             | Drying temperature [°C.] | Drying time [min] | CTL thickness [μm] | $\gamma$ Content [%] | $\delta$ Content [%] | Percentage of $\gamma$ content to $\delta$ content |
|-----------------------------|--------------------------|-------------------|--------------------|----------------------|----------------------|----------------------------------------------------|
| Photosensitive member D-101 | 130                      | 130               | 20                 | 0                    | 0                    | —                                                  |
| Photosensitive member D-102 | 125                      | 60                | 20                 | 0.65                 | 0                    | —                                                  |
| Photosensitive member D-103 | 120                      | 60                | 20                 | 2.11                 | 0                    | —                                                  |
| Photosensitive member D-104 | 125                      | 60                | 20                 | 0                    | 0.13                 | 0                                                  |
| Photosensitive member D-105 | 120                      | 60                | 20                 | 0                    | 1.35                 | 0                                                  |
| Photosensitive member D-106 | 115                      | 45                | 20                 | 2.31                 | 0.09                 | 2567                                               |
| Photosensitive member D-107 | 115                      | 60                | 20                 | 2.12                 | 1.25                 | 170                                                |
| Photosensitive member D-108 | 115                      | 60                | 20                 | 0.78                 | 1.51                 | 52                                                 |
| Photosensitive member D-109 | 115                      | 60                | 20                 | 2.14                 | 1.56                 | 137                                                |

TABLE 18

| Compound                  | $\alpha$ | $\beta$    | (( $\beta$ ) content/ |               | $\gamma$                                              | $\delta$      | Another solvent |                |
|---------------------------|----------|------------|-----------------------|---------------|-------------------------------------------------------|---------------|-----------------|----------------|
|                           |          |            | Parts by mass         | Parts by mass |                                                       |               | Parts by mass   | Parts by mass  |
|                           |          |            | Resin $\beta$         | Resin mass    | ( $\alpha$ ) content/( $\alpha$ content/100) $\times$ | Parts by mass | Compound        | Compound       |
| Photosensitive member E-1 | A-1      | 8 Resin A1 | 10                    | 125           | Xylene                                                | 16            | Cyclopentanone  | 28 Methylal 36 |
| Photosensitive member E-2 | A-1      | 8 Resin A1 | 10                    | 125           | Xylene                                                | 21            | Cyclopentanone  | 23 Methylal 36 |
| Photosensitive member E-3 | A-1      | 8 Resin A1 | 10                    | 125           | Xylene                                                | 16            | Cyclopentanone  | 30 Methylal 36 |
| Photosensitive member E-4 | A-1      | 8 Resin A1 | 10                    | 125           | Xylene                                                | 21            | Cyclopentanone  | 25 Methylal 36 |
| Photosensitive member E-5 | A-1      | 8 Resin A1 | 10                    | 125           | Xylene                                                | 8             | Cyclopentanone  | 38 Methylal 36 |
| Photosensitive member E-6 | A-1      | 8 Resin A1 | 10                    | 125           | Xylene                                                | 14            | Cyclopentanone  | 38 Methylal 36 |
| Photosensitive member E-7 | A-1      | 8 Resin A1 | 10                    | 125           | Xylene                                                | 21            | Cyclopentanone  | 23 Methylal 36 |
| Photosensitive member E-8 | A-1      | 8 Resin A1 | 10                    | 125           | Xylene                                                | 16            | Cyclopentanone  | 30 Methylal 36 |
| Photosensitive member E-9 | A-1      | 8 Resin A1 | 10                    | 125           | Xylene                                                | 16            | Cyclopentanone  | 38 Methylal 36 |

TABLE 19

|                           | Drying temperature [° C.] | Drying time [min] | CTL thickness [μm] | γ Content [%] | δ Content [%] | Percentage of γ content to δ content |
|---------------------------|---------------------------|-------------------|--------------------|---------------|---------------|--------------------------------------|
| Photosensitive member E-1 | 120                       | 60                | 20                 | 0.84          | 0.11          | 764                                  |
| Photosensitive member E-2 | 120                       | 60                | 20                 | 1.31          | 0.06          | 2183                                 |
| Photosensitive member E-3 | 120                       | 60                | 20                 | 0.60          | 0.14          | 429                                  |
| Photosensitive member E-4 | 120                       | 60                | 20                 | 1.30          | 0.11          | 1182                                 |
| Photosensitive member E-5 | 120                       | 60                | 20                 | 0.80          | 0.32          | 250                                  |
| Photosensitive member E-6 | 120                       | 60                | 20                 | 1.24          | 0.31          | 400                                  |
| Photosensitive member E-7 | 125                       | 60                | 20                 | 0.65          | 0.01          | 6861                                 |
| Photosensitive member E-8 | 125                       | 60                | 20                 | 0.40          | 0.04          | 1000                                 |
| Photosensitive member E-9 | 125                       | 60                | 20                 | 0.46          | 0.16          | 288                                  |

TABLE 20

| Compound                    | $\alpha$      | $\beta$       | $((\beta)$                               | $\gamma$ | $\delta$      | Another solvent |               |                |    |          |    |
|-----------------------------|---------------|---------------|------------------------------------------|----------|---------------|-----------------|---------------|----------------|----|----------|----|
|                             | Parts by mass | Parts by mass | content/(\mathbf{\alpha}) content) × 100 | Compound | Parts by mass | Parts by mass   | Parts by mass |                |    |          |    |
| Photosensitive member E-101 | A-1           | 8             | Resin A1                                 | 10       | 125           | Xylene          | 16            | Cyclopentanone | 28 | Methylal | 36 |
| Photosensitive member E-102 | A-1           | 8             | Resin A1                                 | 10       | 125           | Xylene          | 46            | Cyclopentanone | 0  | Methylal | 36 |
| Photosensitive member E-103 | A-1           | 8             | Resin A1                                 | 10       | 125           | Xylene          | 46            | Cyclopentanone | 0  | Methylal | 36 |
| Photosensitive member E-104 | A-1           | 8             | Resin A1                                 | 10       | 125           | Xylene          | 0             | Cyclopentanone | 46 | Methylal | 36 |
| Photosensitive member E-105 | A-1           | 8             | Resin A1                                 | 10       | 125           | Xylene          | 0             | Cyclopentanone | 46 | Methylal | 36 |
| Photosensitive member E-106 | A-1           | 8             | Resin A1                                 | 10       | 125           | Xylene          | 21            | Cyclopentanone | 23 | Methylal | 36 |
| Photosensitive member E-107 | A-1           | 8             | Resin A1                                 | 10       | 125           | Xylene          | 21            | Cyclopentanone | 35 | Methylal | 36 |
| Photosensitive member E-108 | A-1           | 8             | Resin A1                                 | 10       | 125           | Xylene          | 15            | Cyclopentanone | 35 | Methylal | 36 |
| Photosensitive member E-109 | A-1           | 8             | Resin A1                                 | 10       | 125           | Xylene          | 21            | Cyclopentanone | 35 | Methylal | 36 |

TABLE 21

|                             | Drying temperature [° C.] | Drying time [min] | CTL thickness [μm] | γ Content [%] | δ Content [%] | Percentage of γ content to δ content |
|-----------------------------|---------------------------|-------------------|--------------------|---------------|---------------|--------------------------------------|
| Photosensitive member E-101 | 130                       | 130               | 20                 | 0             | 0             | —                                    |
| Photosensitive member E-102 | 125                       | 60                | 20                 | 0.68          | 0             | —                                    |
| Photosensitive member E-103 | 120                       | 60                | 20                 | 2.08          | 0             | —                                    |
| Photosensitive member E-104 | 125                       | 60                | 20                 | 0             | 0.12          | 0                                    |
| Photosensitive member E-105 | 120                       | 60                | 20                 | 0             | 1.24          | 0                                    |
| Photosensitive member E-106 | 115                       | 45                | 20                 | 2.28          | 0.11          | 2073                                 |
| Photosensitive member E-107 | 115                       | 60                | 20                 | 2.2           | 0.13          | 1692                                 |
| Photosensitive member E-108 | 115                       | 60                | 20                 | 0.75          | 1.55          | 48                                   |
| Photosensitive member E-109 | 115                       | 60                | 20                 | 2.16          | 1.54          | 140                                  |

TABLE 22

| Compound                  | $\alpha$      | $\beta$       | $((\beta)$                               | $\gamma$ | $\delta$      | Another solvent |               |               |    |          |    |
|---------------------------|---------------|---------------|------------------------------------------|----------|---------------|-----------------|---------------|---------------|----|----------|----|
|                           | Parts by mass | Parts by mass | content/(\mathbf{\alpha}) content) × 100 | Compound | Parts by mass | Parts by mass   | Parts by mass |               |    |          |    |
| Photosensitive member F-1 | A-1           | 8             | Resin A1                                 | 10       | 125           | Xylene          | 38            | Cyclohexanone | 13 | Methylal | 36 |
| Photosensitive member F-2 | A-1           | 8             | Resin A1                                 | 10       | 125           | Xylene          | 30            | Cyclohexanone | 12 | Methylal | 36 |
| Photosensitive member F-3 | A-1           | 8             | Resin A1                                 | 10       | 125           | Xylene          | 38            | Cyclohexanone | 8  | Methylal | 36 |
| Photosensitive member F-4 | A-1           | 8             | Resin A1                                 | 10       | 125           | Xylene          | 38            | Cyclohexanone | 14 | Methylal | 36 |

TABLE 22-continued

|                           | $\alpha$      | $\beta$       | (( $\beta$ )                               | $\gamma$      | $\delta$        | Another solvent |
|---------------------------|---------------|---------------|--------------------------------------------|---------------|-----------------|-----------------|
|                           | Parts by mass | Parts by mass | content/( $\alpha$ ) content) $\times$ 100 | Parts by mass | Parts by mass   | Parts by mass   |
| Compound                  | Compound      | Resin $\beta$ | Compound                                   | Compound      | Compound        | Compound        |
| Photosensitive member F-5 | A-1           | 8 Resin A1    | 10 125                                     | Xylene 38     | Cyclohexanone 3 | Methylal 36     |
| Photosensitive member F-6 | A-1           | 8 Resin A1    | 10 125                                     | Xylene 28     | Cyclohexanone 5 | Methylal 36     |
| Photosensitive member F-7 | A-1           | 8 Resin A1    | 10 125                                     | Xylene 30     | Cyclohexanone 9 | Methylal 36     |

TABLE 23

|                           | Drying temperature [° C.] | Drying time [min] | CTL thickness [μm] | $\gamma$ Content [%] | $\delta$ Content [%] | Percentage of $\gamma$ content to $\delta$ content |
|---------------------------|---------------------------|-------------------|--------------------|----------------------|----------------------|----------------------------------------------------|
| Photosensitive member F-1 | 120                       | 60                | 20                 | 1.40                 | 0.12                 | 1167                                               |
| Photosensitive member F-2 | 120                       | 60                | 20                 | 0.95                 | 0.14                 | 667                                                |
| Photosensitive member F-3 | 120                       | 60                | 20                 | 0.92                 | 0.40                 | 230                                                |
| Photosensitive member F-4 | 120                       | 60                | 20                 | 1.42                 | 0.38                 | 375                                                |
| Photosensitive member F-5 | 125                       | 60                | 20                 | 0.81                 | 0.01                 | 8550                                               |
| Photosensitive member F-6 | 125                       | 60                | 20                 | 0.47                 | 0.05                 | 1000                                               |
| Photosensitive member F-7 | 125                       | 60                | 20                 | 0.47                 | 0.18                 | 263                                                |

TABLE 24

|                             | $\alpha$      | $\beta$       | (( $\beta$ )                               | $\gamma$      | $\delta$         | Another solvent |
|-----------------------------|---------------|---------------|--------------------------------------------|---------------|------------------|-----------------|
|                             | Parts by mass | Parts by mass | content/( $\alpha$ ) content) $\times$ 100 | Parts by mass | Parts by mass    | Parts by mass   |
| Compound                    | Compound      | Resin $\beta$ | Compound                                   | Compound      | Compound         | Compound        |
| Photosensitive member F-101 | A-1           | 8 Resin A1    | 10 125                                     | Xylene 38     | Cyclohexanone 13 | Methylal 36     |
| Photosensitive member F-102 | A-1           | 8 Resin A1    | 10 125                                     | Xylene 46     | Cyclohexanone 0  | Methylal 36     |
| Photosensitive member F-103 | A-1           | 8 Resin A1    | 10 125                                     | Xylene 46     | Cyclohexanone 0  | Methylal 36     |
| Photosensitive member F-104 | A-1           | 8 Resin A1    | 10 125                                     | Xylene 0      | Cyclohexanone 46 | Methylal 36     |
| Photosensitive member F-105 | A-1           | 8 Resin A1    | 10 125                                     | Xylene 0      | Cyclohexanone 46 | Methylal 36     |
| Photosensitive member F-106 | A-1           | 8 Resin A1    | 10 125                                     | Xylene 43     | Cyclohexanone 3  | Methylal 36     |
| Photosensitive member F-107 | A-1           | 8 Resin A1    | 10 125                                     | Xylene 30     | Cyclohexanone 10 | Methylal 36     |
| Photosensitive member F-108 | A-1           | 8 Resin A1    | 10 125                                     | Xylene 15     | Cyclohexanone 35 | Methylal 36     |
| Photosensitive member F-109 | A-1           | 8 Resin A1    | 10 125                                     | Xylene 35     | Cyclohexanone 10 | Methylal 36     |

TABLE 25

|                             | Drying temperature [° C.] | Drying time [min] | CTL thickness [μm] | $\gamma$ Content [%] | $\delta$ Content [%] | Percentage of $\gamma$ content to $\delta$ content |
|-----------------------------|---------------------------|-------------------|--------------------|----------------------|----------------------|----------------------------------------------------|
| Photosensitive member F-101 | 130                       | 130               | 20                 | 0                    | 0                    | —                                                  |
| Photosensitive member F-102 | 125                       | 60                | 20                 | 0.65                 | 0                    | —                                                  |
| Photosensitive member F-103 | 120                       | 60                | 20                 | 2.11                 | 0                    | —                                                  |
| Photosensitive member F-104 | 130                       | 60                | 20                 | 0                    | 0.13                 | 0                                                  |
| Photosensitive member F-105 | 125                       | 60                | 20                 | 0                    | 1.31                 | 0                                                  |
| Photosensitive member F-106 | 115                       | 45                | 20                 | 2.31                 | 0.09                 | 2567                                               |
| Photosensitive member F-107 | 115                       | 60                | 20                 | 2.12                 | 1.25                 | 170                                                |
| Photosensitive member F-108 | 115                       | 60                | 20                 | 0.78                 | 1.51                 | 52                                                 |
| Photosensitive member F-109 | 115                       | 60                | 20                 | 2.14                 | 1.56                 | 137                                                |

TABLE 26

| Compound                  | $\alpha$      | $\beta$       | $((\beta))$                                              | $\gamma$               | $\delta$               | Another solvent        |                        |                |   |          |    |
|---------------------------|---------------|---------------|----------------------------------------------------------|------------------------|------------------------|------------------------|------------------------|----------------|---|----------|----|
|                           | Parts by mass | Resin $\beta$ | Parts by mass content/( $\alpha$ ) content) $\times$ 100 | Parts by mass Compound | Parts by mass Compound | Parts by mass Compound | Parts by mass Compound |                |   |          |    |
|                           |               |               |                                                          |                        |                        |                        |                        |                |   |          |    |
| Photosensitive member G-1 | A-1           | 8             | Resin A1                                                 | 10                     | 125                    | Toluene                | 42                     | Cyclopentanone | 3 | Methylal | 36 |

TABLE 27

|                           | Drying temperature [° C.] | Drying time [min] | CTL thickness [μm] | $\gamma$ Content [%] | $\delta$ Content [%] | Percentage of $\gamma$ content to $\delta$ content |
|---------------------------|---------------------------|-------------------|--------------------|----------------------|----------------------|----------------------------------------------------|
|                           |                           |                   |                    |                      |                      |                                                    |
| Photosensitive member G-1 | 120                       | 60                | 20                 | 0.10                 | 0.02                 | 500                                                |

TABLE 28

| Compound                    | $\alpha$      | $\beta$       | $((\beta))$                                              | $\gamma$               | $\delta$               | Another solvent        |                        |                |   |          |    |
|-----------------------------|---------------|---------------|----------------------------------------------------------|------------------------|------------------------|------------------------|------------------------|----------------|---|----------|----|
|                             | Parts by mass | Resin $\beta$ | Parts by mass content/( $\alpha$ ) content) $\times$ 100 | Parts by mass Compound | Parts by mass Compound | Parts by mass Compound | Parts by mass Compound |                |   |          |    |
|                             |               |               |                                                          |                        |                        |                        |                        |                |   |          |    |
| Photosensitive member G-101 | A-1           | 8             | Resin A1                                                 | 10                     | 125                    | Toluene                | 45                     | Cyclopentanone | 3 | Methylal | 36 |

TABLE 29

|                             | Drying temperature [° C.] | Drying time [min] | CTL thickness [μm] | $\gamma$ Content [%] | $\delta$ Content [%] | Percentage of $\gamma$ content to $\delta$ content |
|-----------------------------|---------------------------|-------------------|--------------------|----------------------|----------------------|----------------------------------------------------|
|                             |                           |                   |                    |                      |                      |                                                    |
| Photosensitive member G-101 | 125                       | 60                | 20                 | 0                    | 0                    | —                                                  |

## Evaluations of Electrophotographic Photosensitive Members

## Example A-1

Photosensitive member A-1 was installed in the cyan station of a test apparatus modified from Canon electrophotographic apparatus (copy machine) iR-ADV C5255, and examined for the following properties. Potential

For measuring surface potentials (dark portion potential and light portion potential) of the electrophotographic photosensitive member, the cartridge of the above-mentioned test apparatus was modified, and the developing device was replaced with a jig to which a potential measuring probe was fixed so as to lie at a position of 178 mm from the end of the electrophotographic photosensitive member (approximately at the center). The measurement was thus performed at the developing position. Applied bias was controlled so that an unexposed portion of the photoelectric photosensitive member would have a dark portion potential of -700 V, and laser beam was adjusted to 0.15  $\mu$ J/cm<sup>2</sup> at the surface of the photosensitive member. Then, the light portion potential was measured with light attenuated from the dark portion potential under the above-described conditions. The light portion potential was -221 V. Table 30 shows the difference of the light portion potential of each photosensitive member from the lowest absolute value of the light portion potentials of photosensitive members A-101 to A-110. Sensitivity was ranked according to the following criteria:

A: When exhibited a difference of 25 V or more from the light portion potential of the most sensitive photosensitive member of Comparative Examples A-1 to A-10.

B: When exhibited a difference in the range of 15 V to 24 V from the light portion potential of the most sensitive photosensitive member of Comparative Examples A-1 to A-10.

C: When exhibited a difference in the range of 5 V to 14 V from the light portion potential of the most sensitive photosensitive member of Comparative Examples A-1 to A-10.

D: When exhibited a difference of 4 V or less from the light portion potential of the most sensitive photosensitive member of Comparative Examples A-1 to A-10.

## Image Quality

The cyan station of the above-mentioned test apparatus was set, and the initial potential of the electrophotographic photosensitive member was adjusted under the conditions of 23° C. and 50% RH to a dark portion potential (Vd) of -700 V and a light portion potential (V1) of -200 V by controlling the charging device and the image exposure device.

Then, a screen image with a cyan density of 30% was output as a halftone image. No defect in the image was confirmed.

## Examples A-2 to A-35

Photosensitive members A-2 to A-35 were evaluated in the same manner as photosensitive member A-1 of Example 1. The results are shown in Table 30.

## Comparative Examples a-1 to a-10

Photosensitive members A-101 to A-110 were evaluated in the same manner as photosensitive member A-1 of Example A-1. The results are shown in Table 30.

## Examples B-1 to B-30

Photosensitive members B-1 to B-30 were evaluated in the same manner as photosensitive member A-1 of Example A-1. Table 31 shows the difference of the light portion potential of each photosensitive member from the lowest absolute value of the light portion potentials of photosensitive members B-101 to B-110. Sensitivity was ranked according to the following criteria:

- A: When exhibited a difference of 25 V or more from the light portion potential of the most sensitive photosensitive member of Comparative Examples B-1 to B-10.
- B: When exhibited a difference in the range of 15 V to 24 V from the light portion potential of the most sensitive photosensitive member of Comparative Examples B-1 to B-10.
- C: When exhibited a difference in the range of 5 V to 14 V from the light portion potential of the most sensitive photosensitive member of Comparative Examples B-1 to B-10.
- D: When exhibited a difference in the range of 4 V or less from the light portion potential of the most sensitive photosensitive member of Comparative Examples B-1 to B-10.

## Comparative Examples B-1 to B-10

Photosensitive members B-101 to B-110 were evaluated in the same manner as photosensitive member A-1 of Example A-1. The results are shown in Table 31.

## Examples C-1 to C-30

Photosensitive members C-1 to C-30 were evaluated in the same manner as photosensitive member A-1 of Example A-1. Table 32 shows the difference of the light portion potential of each photosensitive member from the lowest absolute value of the light portion potentials of photosensitive members C-101 to C-110. Sensitivity was ranked according to the following criteria:

- A: When exhibited a difference of 25 V or more from the light portion potential of the most sensitive photosensitive member of Comparative Examples C-1 to C-10.
- B: When exhibited a difference in the range of 15 V to 24 V from the light portion potential of the most sensitive photosensitive member of Comparative Examples C-1 to C-10.
- C: When exhibited a difference in the range of 5 V to 14 V from the light portion potential of the most sensitive photosensitive member of Comparative Examples C-1 to C-10.
- D: When exhibited a difference of 4 V or less from the light portion potential of the most sensitive photosensitive member of Comparative Examples C-1 to C-10.

## Comparative Examples C-1 to C-10

Photosensitive members C-101 to C-110 were evaluated in the same manner as photosensitive member A-1 of Example A-1. The results are shown in Table 32.

## Examples D-1 to D-9

Photosensitive members D-1 to D-9 were evaluated in the same manner as photosensitive member A-1 of Example A-1. Table 33 shows the difference of the light portion potential of

each photosensitive member from the lowest absolute value of the light portion potentials of photosensitive members D-101 to D-109. Sensitivity was ranked according to the following criteria:

- 5 A: When exhibited a difference of 25 V or more from the light portion potential of the most sensitive photosensitive member of Comparative Examples D-1 to D-9.
- B: When exhibited a difference in the range of 15 V to 24 V from the light portion potential of the most sensitive photosensitive member of Comparative Examples D-1 to D-9.
- C: When exhibited a difference in the range of 5 V to 14 V from the light portion potential of the most sensitive photosensitive member of Comparative Examples D-1 to D-9.
- D: When exhibited a difference of 4 V or less from the light portion potential of the most sensitive photosensitive member of Comparative Examples D-1 to D-9.

## Comparative Examples D-1 to D-9

Photosensitive members D-101 to D-109 were evaluated in the same manner as photosensitive member A-1 of Example A-1. The results are shown in Table 33.

## Comparative Example D-10

Photosensitive member D-110 was evaluated in the same manner as photosensitive member A-1 of Example A-1. The light portion potential was -415 V, and the difference from the light portion potential of the most sensitive member of Comparative Examples D-1 to D-9 was -10 V.

## Comparative Example D-11

- 35 Photosensitive member D-111 was evaluated in the same manner as photosensitive member A-1 of Example A-1. The light portion potential was -413 V, and the difference from the light portion potential of the most sensitive member of Comparative Examples D-1 to D-9 was -7 V.

## Examples E-1 to E-9

Photosensitive members E-1 to E-9 were evaluated in the same manner as photosensitive member A-1 of Example A-1. Table 34 shows the difference of the light portion potential of each photosensitive member from the lowest absolute value of the light portion potentials of photosensitive members E-101 to E-109. Sensitivity was ranked according to the following criteria:

- 45 A: When exhibited a difference of 25 V or more from the light portion potential of the most sensitive photosensitive member of Comparative Examples E-1 to E-9.
- B: When exhibited a difference in the range of 15 V to 24 V from the light portion potential of the most sensitive photosensitive member of Comparative Examples E-1 to E-9.
- C: When exhibited a difference in the range of 5 V to 14 V from the light portion potential of the most sensitive photosensitive member of Comparative Examples E-1 to E-9.
- D: When exhibited a difference of 4 V or less from the light portion potential of the most sensitive photosensitive member of Comparative Examples E-1 to E-9.

## Comparative Examples E-1 to E-9

Photosensitive members E-101 to E-109 were evaluated in the same manner as photosensitive member A-1 of Example A-1. The results are shown in Table 34.

Photosensitive members F-1 to F-7 were evaluated in the same manner as photosensitive member A-1 of Example A-1. Table 35 shows the difference of the light portion potential of each photosensitive member from the lowest absolute value of the light portion potentials of photosensitive members F-101 to F-109. Sensitivity was ranked according to the following criteria:

- A: When exhibited a difference of 25 V or more from the light portion potential of the most sensitive photosensitive member of Comparative Examples F-1 to F-9.
- B: When exhibited a difference in the range of 15 V to 24 V from the light portion potential of the most sensitive photosensitive member of Comparative Examples F-1 to F-9.
- C: When exhibited a difference in the range of 5 V to 14 V from the light portion potential of the most sensitive photosensitive member of Comparative Examples F-1 to F-9.
- D: When exhibited a difference of 4 V or less from the light portion potential of the most sensitive photosensitive member of Comparative Examples F-1 to F-9.

## Comparative Examples F-1 to F-9

Photosensitive members F-101 to F-109 were evaluated in the same manner as photosensitive member A-1 of Example A-1. The results are shown in Table 35.

Photosensitive member G-1 was evaluated in the same manner as photosensitive member A-1 of Example A-1. Table 36 shows the difference in light portion potential from photosensitive member G-101. Sensitivity was ranked according to the following criteria:

- A: When exhibited a difference of 25 V or more from Comparative Example G-101.
- B: When exhibited a difference in the range of 15 V to 24 V from Comparative Example G-101.
- C: When exhibited a difference in the range of 5 V to 14 V from Comparative Example G-101.
- D: When exhibited a difference of 4 V or less from Comparative Example G-101.

## Comparative Example G-1

Photosensitive member G-101 was evaluated in the same manner as photosensitive member A-1 of Example A-1. The results are shown in Table 36.

TABLE 30

|                          |                             | Light portion potential [V] | Difference | Rank |
|--------------------------|-----------------------------|-----------------------------|------------|------|
| Example A-1              | Photosensitive member A-1   | -221                        | 27         | A    |
| Example A-2              | Photosensitive member A-2   | -218                        | 30         | A    |
| Example A-3              | Photosensitive member A-3   | -223                        | 25         | A    |
| Example A-4              | Photosensitive member A-4   | -217                        | 31         | A    |
| Example A-5              | Photosensitive member A-5   | -223                        | 25         | A    |
| Example A-6              | Photosensitive member A-6   | -220                        | 28         | A    |
| Example A-7              | Photosensitive member A-7   | -238                        | 10         | C    |
| Example A-8              | Photosensitive member A-8   | -229                        | 19         | B    |
| Example A-9              | Photosensitive member A-9   | -228                        | 20         | B    |
| Example A-10             | Photosensitive member A-10  | -213                        | 35         | A    |
| Example A-11             | Photosensitive member A-11  | -227                        | 21         | B    |
| Example A-12             | Photosensitive member A-12  | -231                        | 17         | B    |
| Example A-13             | Photosensitive member A-13  | -221                        | 27         | A    |
| Example A-14             | Photosensitive member A-14  | -228                        | 20         | B    |
| Example A-15             | Photosensitive member A-15  | -235                        | 13         | C    |
| Example A-16             | Photosensitive member A-16  | -221                        | 27         | A    |
| Example A-17             | Photosensitive member A-17  | -230                        | 18         | B    |
| Example A-18             | Photosensitive member A-18  | -236                        | 12         | C    |
| Example A-19             | Photosensitive member A-19  | -227                        | 21         | B    |
| Example A-20             | Photosensitive member A-20  | -232                        | 16         | B    |
| Example A-21             | Photosensitive member A-21  | -229                        | 19         | B    |
| Example A-22             | Photosensitive member A-22  | -230                        | 18         | B    |
| Example A-23             | Photosensitive member A-23  | -228                        | 20         | B    |
| Example A-24             | Photosensitive member A-24  | -233                        | 15         | B    |
| Example A-25             | Photosensitive member A-25  | -232                        | 16         | B    |
| Example A-26             | Photosensitive member A-26  | -239                        | 9          | C    |
| Example A-27             | Photosensitive member A-27  | -238                        | 10         | C    |
| Example A-28             | Photosensitive member A-28  | -236                        | 12         | C    |
| Example A-29             | Photosensitive member A-29  | -240                        | 8          | C    |
| Example A-30             | Photosensitive member A-30  | -243                        | 5          | C    |
| Example A-31             | Photosensitive member A-31  | -223                        | 25         | A    |
| Example A-32             | Photosensitive member A-32  | -222                        | 26         | A    |
| Example A-33             | Photosensitive member A-33  | -220                        | 28         | A    |
| Example A-34             | Photosensitive member A-34  | -218                        | 30         | A    |
| Example A-35             | Photosensitive member A-35  | -220                        | 28         | A    |
| Comparative Example A-1  | Photosensitive member A-101 | -255                        | -7         | D    |
| Comparative Example A-2  | Photosensitive member A-102 | -250                        | -2         | D    |
| Comparative Example A-3  | Photosensitive member A-103 | -248                        | 0          | D    |
| Comparative Example A-4  | Photosensitive member A-104 | -250                        | -2         | D    |
| Comparative Example A-5  | Photosensitive member A-105 | -265                        | -17        | D    |
| Comparative Example A-6  | Photosensitive member A-106 | -260                        | -12        | D    |
| Comparative Example A-7  | Photosensitive member A-107 | -251                        | -3         | D    |
| Comparative Example A-8  | Photosensitive member A-108 | -253                        | -5         | D    |
| Comparative Example A-9  | Photosensitive member A-109 | -250                        | -2         | D    |
| Comparative Example A-10 | Photosensitive member A-110 | -255                        | -7         | D    |

TABLE 31

|                          |                             | Light portion<br>potential [V] | Difference | Rank |
|--------------------------|-----------------------------|--------------------------------|------------|------|
| Example B-1              | Photosensitive member B-1   | -243                           | 28         | A    |
| Example B-2              | Photosensitive member B-2   | -241                           | 30         | A    |
| Example B-3              | Photosensitive member B-3   | -242                           | 29         | A    |
| Example B-4              | Photosensitive member B-4   | -243                           | 28         | A    |
| Example B-5              | Photosensitive member B-5   | -241                           | 30         | A    |
| Example B-6              | Photosensitive member B-6   | -241                           | 30         | A    |
| Example B-7              | Photosensitive member B-7   | -262                           | 9          | C    |
| Example B-8              | Photosensitive member B-8   | -250                           | 21         | B    |
| Example B-9              | Photosensitive member B-9   | -249                           | 22         | B    |
| Example B-10             | Photosensitive member B-10  | -238                           | 33         | A    |
| Example B-11             | Photosensitive member B-11  | -254                           | 17         | B    |
| Example B-12             | Photosensitive member B-12  | -251                           | 20         | B    |
| Example B-13             | Photosensitive member B-13  | -244                           | 27         | A    |
| Example B-14             | Photosensitive member B-14  | -253                           | 18         | B    |
| Example B-15             | Photosensitive member B-15  | -261                           | 10         | C    |
| Example B-16             | Photosensitive member B-16  | -243                           | 28         | A    |
| Example B-17             | Photosensitive member B-17  | -255                           | 16         | B    |
| Example B-18             | Photosensitive member B-18  | -264                           | 7          | C    |
| Example B-19             | Photosensitive member B-19  | -256                           | 15         | B    |
| Example B-20             | Photosensitive member B-20  | -253                           | 18         | B    |
| Example B-21             | Photosensitive member B-21  | -265                           | 6          | B    |
| Example B-22             | Photosensitive member B-22  | -254                           | 17         | B    |
| Example B-23             | Photosensitive member B-23  | -255                           | 16         | B    |
| Example B-24             | Photosensitive member B-24  | -250                           | 21         | B    |
| Example B-25             | Photosensitive member B-25  | -256                           | 15         | B    |
| Example B-26             | Photosensitive member B-26  | -263                           | 8          | C    |
| Example B-27             | Photosensitive member B-27  | -265                           | 6          | C    |
| Example B-28             | Photosensitive member B-28  | -260                           | 11         | C    |
| Example B-29             | Photosensitive member B-29  | -263                           | 8          | C    |
| Example B-30             | Photosensitive member B-30  | -264                           | 7          | C    |
| Comparative Example B-1  | Photosensitive member B-101 | -255                           | -7         | D    |
| Comparative Example B-2  | Photosensitive member B-102 | -250                           | -2         | D    |
| Comparative Example B-3  | Photosensitive member B-103 | -248                           | 0          | D    |
| Comparative Example B-4  | Photosensitive member B-104 | -250                           | -2         | D    |
| Comparative Example B-5  | Photosensitive member B-105 | -265                           | -17        | D    |
| Comparative Example B-6  | Photosensitive member B-106 | -260                           | -12        | D    |
| Comparative Example B-7  | Photosensitive member B-107 | -251                           | -3         | D    |
| Comparative Example B-8  | Photosensitive member B-108 | -253                           | -5         | D    |
| Comparative Example B-9  | Photosensitive member B-109 | -250                           | -2         | D    |
| Comparative Example B-10 | Photosensitive member B-110 | -255                           | -7         | D    |

TABLE 32

|              |                            | Light portion<br>potential [V] | Difference | Rank |
|--------------|----------------------------|--------------------------------|------------|------|
| Example C-1  | Photosensitive member C-1  | -202                           | 29         | A    |
| Example C-2  | Photosensitive member C-2  | -203                           | 28         | A    |
| Example C-3  | Photosensitive member C-3  | -204                           | 27         | A    |
| Example C-4  | Photosensitive member C-4  | -198                           | 33         | A    |
| Example C-5  | Photosensitive member C-5  | -202                           | 29         | A    |
| Example C-6  | Photosensitive member C-6  | -198                           | 33         | A    |
| Example C-7  | Photosensitive member C-7  | -220                           | 11         | C    |
| Example C-8  | Photosensitive member C-8  | -215                           | 16         | B    |
| Example C-9  | Photosensitive member C-9  | -212                           | 19         | B    |
| Example C-10 | Photosensitive member C-10 | -195                           | 36         | A    |
| Example C-11 | Photosensitive member C-11 | -211                           | 20         | B    |
| Example C-12 | Photosensitive member C-12 | -216                           | 15         | B    |
| Example C-13 | Photosensitive member C-13 | -201                           | 30         | A    |
| Example C-14 | Photosensitive member C-14 | -213                           | 18         | B    |
| Example C-15 | Photosensitive member C-15 | -220                           | 11         | C    |
| Example C-16 | Photosensitive member C-16 | -205                           | 26         | A    |
| Example C-17 | Photosensitive member C-17 | -213                           | 18         | B    |
| Example C-18 | Photosensitive member C-18 | -220                           | 11         | C    |
| Example C-19 | Photosensitive member C-19 | -211                           | 20         | B    |
| Example C-20 | Photosensitive member C-20 | -212                           | 19         | B    |
| Example C-21 | Photosensitive member C-21 | -210                           | 21         | B    |
| Example C-22 | Photosensitive member C-22 | -215                           | 16         | B    |
| Example C-23 | Photosensitive member C-23 | -213                           | 18         | B    |
| Example C-24 | Photosensitive member C-24 | -213                           | 18         | B    |
| Example C-25 | Photosensitive member C-25 | -210                           | 21         | B    |
| Example C-26 | Photosensitive member C-26 | -220                           | 11         | C    |
| Example C-27 | Photosensitive member C-27 | -221                           | 10         | C    |
| Example C-28 | Photosensitive member C-28 | -226                           | 5          | C    |

TABLE 32-continued

|                          |                             | Light portion<br>potential [V] | Difference | Rank |
|--------------------------|-----------------------------|--------------------------------|------------|------|
| Example C-29             | Photosensitive member C-29  | -225                           | 6          | C    |
| Example C-30             | Photosensitive member C-30  | -218                           | 13         | C    |
| Comparative Example C-1  | Photosensitive member C-101 | -235                           | -4         | D    |
| Comparative Example C-2  | Photosensitive member C-102 | -233                           | -2         | D    |
| Comparative Example C-3  | Photosensitive member C-103 | -231                           | 0          | D    |
| Comparative Example C-4  | Photosensitive member C-104 | -231                           | 0          | D    |
| Comparative Example C-5  | Photosensitive member C-105 | -241                           | -10        | D    |
| Comparative Example C-6  | Photosensitive member C-106 | -236                           | -5         | D    |
| Comparative Example C-7  | Photosensitive member C-107 | -233                           | -2         | D    |
| Comparative Example C-8  | Photosensitive member C-108 | -235                           | -4         | D    |
| Comparative Example C-9  | Photosensitive member C-109 | -232                           | -1         | D    |
| Comparative Example C-10 | Photosensitive member C-110 | -234                           | -3         | D    |

TABLE 33

|                          |                             | Light portion<br>potential [V] | Difference | Rank |
|--------------------------|-----------------------------|--------------------------------|------------|------|
| Example D-1              | Photosensitive member D-1   | -378                           | 27         | A    |
| Example D-2              | Photosensitive member D-2   | -375                           | 30         | A    |
| Example D-3              | Photosensitive member D-3   | -376                           | 29         | A    |
| Example D-4              | Photosensitive member D-4   | -373                           | 32         | A    |
| Example D-5              | Photosensitive member D-5   | -380                           | 25         | A    |
| Example D-6              | Photosensitive member D-6   | -377                           | 28         | A    |
| Example D-7              | Photosensitive member D-7   | -373                           | 32         | A    |
| Example D-8              | Photosensitive member D-8   | -380                           | 25         | A    |
| Example D-9              | Photosensitive member D-9   | -380                           | 25         | A    |
| Comparative Example D-1  | Photosensitive member D-101 | -410                           | -5         | D    |
| Comparative Example D-2  | Photosensitive member D-102 | -405                           | 0          | D    |
| Comparative Example D-3  | Photosensitive member D-103 | -405                           | 0          | D    |
| Comparative Example D-4  | Photosensitive member D-104 | -406                           | -1         | D    |
| Comparative Example D-5  | Photosensitive member D-105 | -414                           | -9         | D    |
| Comparative Example D-6  | Photosensitive member D-106 | -408                           | -3         | D    |
| Comparative Example D-7  | Photosensitive member D-107 | -407                           | -2         | D    |
| Comparative Example D-8  | Photosensitive member D-108 | -409                           | -4         | D    |
| Comparative Example D-9  | Photosensitive member D-109 | -413                           | -8         | D    |
| Comparative Example D-10 | Photosensitive member D-110 | -418                           | -13        | D    |

TABLE 34

|                         |                             | Light portion<br>potential [V] | Difference | Rank |
|-------------------------|-----------------------------|--------------------------------|------------|------|
| Example E-1             | Photosensitive member E-1   | -379                           | 29         | A    |
| Example E-2             | Photosensitive member E-2   | -378                           | 30         | A    |
| Example E-3             | Photosensitive member E-3   | -381                           | 27         | A    |
| Example E-4             | Photosensitive member E-4   | -377                           | 31         | A    |
| Example E-5             | Photosensitive member E-5   | -383                           | 25         | A    |
| Example E-6             | Photosensitive member E-6   | -377                           | 31         | A    |
| Example E-7             | Photosensitive member E-7   | -376                           | 32         | A    |
| Example E-8             | Photosensitive member E-8   | -378                           | 30         | A    |
| Example E-9             | Photosensitive member E-9   | -375                           | 33         | A    |
| Comparative Example E-1 | Photosensitive member E-101 | -418                           | -10        | D    |
| Comparative Example E-2 | Photosensitive member E-102 | -408                           | 0          | D    |
| Comparative Example E-3 | Photosensitive member E-103 | -409                           | -1         | D    |
| Comparative Example E-4 | Photosensitive member E-104 | -413                           | -5         | D    |
| Comparative Example E-5 | Photosensitive member E-105 | -412                           | -4         | D    |
| Comparative Example E-6 | Photosensitive member E-106 | -414                           | -6         | D    |
| Comparative Example E-7 | Photosensitive member E-107 | -411                           | -3         | D    |
| Comparative Example E-8 | Photosensitive member E-108 | -415                           | -7         | D    |
| Comparative Example E-9 | Photosensitive member E-109 | -423                           | -15        | D    |

TABLE 35

|             |                           | Light portion<br>potential [V] | Difference | Rank |
|-------------|---------------------------|--------------------------------|------------|------|
| Example F-1 | Photosensitive member F-1 | -410                           | 14         | C    |
| Example F-2 | Photosensitive member F-2 | -412                           | 12         | C    |
| Example F-3 | Photosensitive member F-3 | -414                           | 10         | C    |

TABLE 35-continued

|                         |                             | Light portion potential [V] | Difference | Rank |
|-------------------------|-----------------------------|-----------------------------|------------|------|
| Example F-4             | Photosensitive member F-4   | -417                        | 7          | C    |
| Example F-5             | Photosensitive member F-5   | -415                        | 9          | C    |
| Example F-6             | Photosensitive member F-6   | -413                        | 11         | C    |
| Example F-7             | Photosensitive member F-7   | -411                        | 13         | C    |
| Comparative Example F-1 | Photosensitive member F-101 | -428                        | -4         | D    |
| Comparative Example F-2 | Photosensitive member F-102 | -424                        | 0          | D    |
| Comparative Example F-3 | Photosensitive member F-103 | -426                        | -2         | D    |
| Comparative Example F-4 | Photosensitive member F-104 | -433                        | -9         | D    |
| Comparative Example F-5 | Photosensitive member F-105 | -431                        | -7         | D    |
| Comparative Example F-6 | Photosensitive member F-106 | -427                        | -3         | D    |
| Comparative Example F-7 | Photosensitive member F-107 | -431                        | -7         | D    |
| Comparative Example F-8 | Photosensitive member F-108 | -428                        | -4         | D    |
| Comparative Example F-9 | Photosensitive member F-109 | -440                        | -16        | D    |

TABLE 36

|                         |                             | Light portion potential [V] | Difference | Rank |
|-------------------------|-----------------------------|-----------------------------|------------|------|
| Example G-1             | Photosensitive member G-1   | -398                        | 13         | C    |
| Comparative Example G-1 | Photosensitive member G-101 | -411                        | 0          | D    |

25

### Preparation of Photosensitive Members H-1 to H-3 and H-101 to H-103

Electrophotographic photosensitive members were prepared in the same process as photosensitive member A-1, except that resin  $\beta$  and the contents of compounds  $\gamma$  and  $\gamma$  were varied according to Table 37 and that the drying tem-

perature and drying time were set as shown in Table 38. Details are shown in Tables 37 and 38. The resulting electrophotographic photosensitive members were evaluated as photosensitive members H-1 to H-3 and H-101 to H-103, respectively.

TABLE 37

| Compound                    | $\alpha$      | $\beta$       | $(\beta)$                                  | $\gamma$      | $\delta$      | Another solvent |               |                              |      |          |    |
|-----------------------------|---------------|---------------|--------------------------------------------|---------------|---------------|-----------------|---------------|------------------------------|------|----------|----|
|                             | Parts by mass | Parts by mass | content/( $\alpha$ ) content) $\times$ 100 | Parts by mass | Parts by mass | Parts by mass   | Parts by mass |                              |      |          |    |
|                             |               | $\beta$       |                                            | Compound      | Compound      | Compound        | Compound      |                              |      |          |    |
| Photosensitive member H-1   | A-1/A-2       | 7.2/0.8       | Resin B2                                   | 10            | 125           | Xylene          | 16            | Cyclopentanone/Cyclohexanone | 24/4 | Methylal | 36 |
| Photosensitive member H-2   | A-1/A-2       | 7.2/0.8       | Resin B2                                   | 10            | 125           | Xylene/Toluene  | 5/11          | Cyclopentanone               | 28   | Methylal | 36 |
| Photosensitive member H-3   | A-1/A-2       | 7.2/0.8       | Resin B2                                   | 10            | 125           | Xylene/Toluene  | 5/11          | Cyclopentanone/Cyclohexanone | 24/4 | Methylal | 36 |
| Photosensitive member H-101 | A-1/A-2       | 7.2/0.8       | Resin B2                                   | 10            | 125           | Xylene          | 46            | Cyclopentanone               | 0    | Methylal | 36 |
| Photosensitive member H-102 | A-1/A-2       | 7.2/0.8       | Resin B2                                   | 10            | 125           | Xylene          | 0             | Cyclopentanone               | 46   | Methylal | 36 |
| Photosensitive member H-103 | A-1/A-2       | 7.2/0.8       | Resin B2                                   | 10            | 125           | Toluene         | 46            | Cyclohexanone                | 0    | Methylal | 36 |
| Photosensitive member H-104 | A-1/A-2       | 7.2/0.8       | Resin B2                                   | 10            | 125           | Toluene         | 0             | Cyclohexanone                | 46   | Methylal | 36 |

TABLE 38

|                             | Drying temperature [ $^{\circ}$ C.] | Drying time [min] | CTL thickness [ $\mu$ m] | $\gamma$ Content [%] | $\delta$ Content [%] | Percentage of $\gamma$ content to $\delta$ content |
|-----------------------------|-------------------------------------|-------------------|--------------------------|----------------------|----------------------|----------------------------------------------------|
| Photosensitive member H-1   | 120                                 | 60                | 30                       | 1.32                 | 0.32/0.29            | 216                                                |
| Photosensitive member H-2   | 120                                 | 60                | 30                       | 0.58/0.46            | 0.20                 | 520                                                |
| Photosensitive member H-3   | 120                                 | 60                | 30                       | 0.74/0.62            | 0.26/0.19            | 302                                                |
| Photosensitive member H-101 | 120                                 | 90                | 30                       | 1.75                 | 0                    | —                                                  |
| Photosensitive member H-102 | 125                                 | 60                | 30                       | 0                    | 0.22                 | 0                                                  |
| Photosensitive member H-103 | 120                                 | 60                | 30                       | 0.43                 | 0                    | —                                                  |
| Photosensitive member H-104 | 130                                 | 60                | 30                       | 0                    | 1.18                 | 0                                                  |

57

## Examples H-1 to H-3

Photosensitive members H-1 to H-3 were evaluated in the same manner as photosensitive member A-1 of Example A-1. The results are shown in Table 39. Sensitivity was ranked according to the following criteria:

- A: When exhibited a difference of 25 V or more from the light portion potential of the most sensitive photosensitive member of Comparative Examples H-1 to H-4.
- B: When exhibited a difference in the range of 15 V to 24 V from the light portion potential of the most sensitive photosensitive member of Comparative Examples H-1 to H-4.
- C: When exhibited a difference in the range of 5 V to 14 V from the light portion potential of the most sensitive photosensitive member of Comparative Examples H-1 to H-4.
- D: When exhibited a difference of 4 V or less from the light portion potential of the most sensitive photosensitive member of Comparative Examples H-1 to H-4.

## Comparative Examples H-1 to H-4

Photosensitive members H-101 to H-104 were evaluated in the same manner as photosensitive member A-1 of Example A-1. The results are shown in Table 39.

TABLE 39

|                         |                             | Light portion potential [V] | Difference | Rank |
|-------------------------|-----------------------------|-----------------------------|------------|------|
| Example H-1             | Photosensitive member H-1   | -225                        | 20         | B    |
| Example H-2             | Photosensitive member H-2   | -231                        | 14         | B    |
| Example H-3             | Photosensitive member H-3   | -228                        | 17         | B    |
| Comparative Example H-1 | Photosensitive member H-101 | -245                        | 0          | D    |
| Comparative Example H-2 | Photosensitive member H-102 | -258                        | -13        | D    |
| Comparative Example H-3 | Photosensitive member H-103 | -248                        | -3         | D    |
| Comparative Example H-4 | Photosensitive member H-104 | -263                        | -18        | D    |

The present disclosure provides a more highly sensitive electrophotographic photosensitive member, and a process cartridge and an electrophotographic apparatus each including the electrophotographic photosensitive member.

While the present invention has been described with reference to exemplary embodiments, it is to be understood that the invention is not limited to the disclosed exemplary embodiments. The scope of the following claims is to be accorded the broadest interpretation so as to encompass all such modifications and equivalent structures and functions.

This application claims the benefit of Japanese Patent Application No. 2014-229323 filed Nov. 11, 2014, and No. 2015-206608 filed Oct. 20, 2015, which are hereby incorporated by reference herein in their entirety.

What is claimed is:

1. An electrophotographic photosensitive member comprising:
  - a support member; and
  - a charge generating layer and a charge transport layer that are disposed over the support member;
  - wherein the charge transport layer contains:
    - (α) a charge transporting compound;
    - (β) a binding resin in a proportion in the range of 50% by mass to 200% by mass relative to the mass of the charge transporting compound;
    - (γ) a compound being at least one of xylene and toluene with a content in the range of 0.01% by mass to 2.00% by mass relative to the total mass of the charge transport layer, and

58

(δ) a cycloalkanone with a content in the range of 0.01% by mass to 1.20% by mass relative to the total mass of the charge transport layer.

2. The electrophotographic photosensitive member according to claim 1, wherein the charge transporting compound has a diphenylamine structure.

3. The electrophotographic photosensitive member according to claim 1, wherein the cycloalkanone contains at least one of cyclopentanone and cyclohexanone.

4. The electrophotographic photosensitive member according to claim 1, wherein the cycloalkanone contains 50% by mass to 100% by mass of cyclopentanone.

5. The electrophotographic photosensitive member according to claim 1, wherein the compound of (γ) contains 50% by mass to 100% by mass of xylene.

6. The electrophotographic photosensitive member according to claim 1, wherein the content of the compound of (γ) in the charge transport layer is in the range of 0.01% by mass to 1.50% by mass relative to the total mass of the charge transport layer.

7. The electrophotographic photosensitive member according to claim 1, wherein the content of the cycloalkanone in the charge transport layer is in the range of 0.01% by mass to 0.80% by mass relative to the total mass of the charge transport layer.

8. The electrophotographic photosensitive member according to claim 1, wherein the content of the compound of (γ) in the charge transport layer is in the range of 200% by mass to 9000% by mass relative to the content of the cycloalkanone in the charge transport layer.

9. The electrophotographic photosensitive member according to claim 1, wherein the charge transporting compound contains a compound expressed by the following general formula (B):



55 wherein Ph<sup>1</sup> and Ph<sup>2</sup> each represent substituted or unsubstituted phenyl, and Ar represents substituted or unsubstituted aryl.

10. The electrophotographic photosensitive member according to claim 1, wherein the charge generating layer contains hydroxy gallium phthalocyanine.

11. The electrophotographic photosensitive member according to claim 1, wherein the charge transport layer has a thickness in the range of 6  $\mu\text{m}$  to 40  $\mu\text{m}$ .

12. The electrophotographic photosensitive member according to claim 1, further comprising at least one additional charge transport layer not containing the compound of (γ) or the cycloalkanone, wherein the thickness of the charge

## 59

transport layer containing the compound of (γ) and the cycloalkanone accounts for 60% or more of the total thickness of the charge transport layers.

13. The electrophotographic photosensitive member according to claim 1, wherein the binding resin is at least one selected from the group consisting of polyester resins and polycarbonate resins.

14. A process cartridge capable of being removably attached to an electrophotographic apparatus, the process cartridge comprising:

an electrophotographic photosensitive member including a support member, and a charge generating layer and a charge transport layer that are disposed over the support member; and

at least one device selected from the group consisting of a charging device, a developing device, a transfer device, and a cleaning device, the at least one device being held with the electrophotographic photosensitive member in one body,

wherein the charge transport layer contains:

(α) a charge transporting compound;

(β) a binding resin in a proportion in the range of 50% by mass to 200% by mass relative to the mass of the charge transporting compound;

(γ) a compound being at least one of xylene and toluene with a content in the range of 0.01% by mass to 2.00% by mass relative to the total mass of the charge transport layer; and

(δ) a cycloalkanone with a content in the range of 0.01% by mass to 1.20% by mass relative to the total mass of the charge transport layer.

15. The process cartridge according to claim 14, wherein the cycloalkanone contains at least one of cyclopentanone and cyclohexanone.

## 60

16. The process cartridge according to claim 15, wherein the cycloalkanone contains 50% by mass to 100% by mass of cyclopentanone.

17. The process cartridge according to claim 14, wherein the compound of (γ) contains 50% by mass to 100% by mass of xylene.

18. An electrophotographic apparatus comprising: an electrophotographic photosensitive member including a support member, and a charge generating layer and a charge transport layer that are disposed over the support member;

a charging device;

an exposure device;

a developing device; and

a transfer divide,

wherein the charge transport layer contains:

(α) a charge transporting compound;

(β) a binding resin in a proportion in the range of 50% by mass to 200% by mass relative to the mass of the charge transporting compound;

(γ) a compound being at least one of xylene and toluene with a content in the range of 0.01% by mass to 2.00% by mass relative to the total mass of the charge transport layer, and

(δ) a cycloalkanone with a content in the range of 0.01% by mass to 1.20% by mass relative to the total mass of the charge transport layer.

19. The electrophotographic apparatus according to claim 18, wherein the cycloalkanone contains at least one of cyclopentanone and cyclohexanone.

20. The electrophotographic apparatus according to claim 19, wherein the cycloalkanone contains 50% by mass to 100% by mass of cyclopentanone.

\* \* \* \* \*